



US012291818B2

(12) **United States Patent**  
**Agresti et al.**

(10) **Patent No.:** **US 12,291,818 B2**  
(45) **Date of Patent:** **May 6, 2025**

(54) **PROCESS AND APPARATUS FOR  
MANUFACTURING A METALLIC  
REINFORCING CORD FOR TYRES FOR  
VEHICLE WHEELS**

(71) Applicant: **Pirelli Tyre S.p.A.**, Milan (IT)

(72) Inventors: **Simone Agresti**, Milan (IT); **Guido Luigi Daghini**, Milan (IT); **Thomas Hanel**, Milan (IT)

(73) Assignee: **PIRELLI TYRE S.p.A.**, Milan (IT)

(\*) Notice: Subject to any disclaimer, the term of this patent is extended or adjusted under 35 U.S.C. 154(b) by 0 days.

(21) Appl. No.: **17/757,065**

(22) PCT Filed: **Dec. 16, 2020**

(86) PCT No.: **PCT/IB2020/062006**

§ 371 (c)(1),  
(2) Date: **Jun. 8, 2022**

(87) PCT Pub. No.: **WO2021/124133**

PCT Pub. Date: **Jun. 24, 2021**

(65) **Prior Publication Data**

US 2023/0002968 A1 Jan. 5, 2023

(30) **Foreign Application Priority Data**

Dec. 17, 2019 (IT) ..... 102019000024280

(51) **Int. Cl.**  
**D07B 1/06** (2006.01)

(52) **U.S. Cl.**  
CPC ..... **D07B 1/062** (2013.01); **D07B 2201/104** (2013.01); **D07B 2205/3021** (2013.01); **D07B 2401/201** (2013.01); **D07B 2501/2046** (2013.01)

(58) **Field of Classification Search**  
CPC ..... D02G 3/406; D02G 3/48; D07B 1/062;  
D07B 1/0646; D07B 2201/104; D07B  
2501/2046  
See application file for complete search history.

(56) **References Cited**

U.S. PATENT DOCUMENTS

1,815,779 A \* 7/1931 Koref ..... H01K 3/02  
117/921  
2,387,320 A \* 10/1945 Foster ..... D02G 3/326  
57/247

(Continued)

FOREIGN PATENT DOCUMENTS

CN 1165221 A 11/1997  
CN 1229866 A 9/1999  
(Continued)

OTHER PUBLICATIONS

Notification of the First Office Action dated Feb. 15, 2023, from China National Intellectual Property Administration, in counterpart Chinese Application No. 202080086028.5.

(Continued)

*Primary Examiner* — Bao-Thieu L Nguyen

(74) *Attorney, Agent, or Firm* — Finnegan, Henderson, Farabow, Garrett & Dunner, L.L.P.

(57) **ABSTRACT**

The present disclosure relates to a process and apparatus for manufacturing a metallic reinforcing cord for tyres for vehicle wheels comprising providing at least one elongated element comprising at least one metallic wire twisted together with at least one textile yarn and removing the at least one textile yarn from the at least one elongated element to form the aforementioned metallic reinforcing cord a wherein the metallic reinforcing cord has a helical geometry, consisting of the at least one metallic wire that extends along a helical path.

**12 Claims, 22 Drawing Sheets**



(56)

## References Cited

## U.S. PATENT DOCUMENTS

|                   |         |                    |              |    |                   |         |
|-------------------|---------|--------------------|--------------|----|-------------------|---------|
| 3,399,521 A *     | 9/1968  | Thoma .....        | D02G 1/00    | CN | 102369321 A       | 3/2012  |
|                   |         |                    | 8/151.2      | CN | 102471998 A       | 5/2012  |
| 4,197,894 A       | 4/1980  | Boileau            |              | CN | 102639337 A       | 8/2012  |
| 4,333,306 A       | 6/1982  | Fumio et al.       |              | CN | 102666133 A       | 9/2012  |
| 4,334,215 A       | 6/1982  | Frazier et al.     |              | CN | 102971459 A       | 3/2013  |
| 4,606,392 A       | 8/1986  | Weidenhaupt et al. |              | CN | 103025543 A       | 4/2013  |
| 4,718,470 A       | 1/1988  | Kusakabe et al.    |              | CN | 203498695 A       | 3/2014  |
| 4,836,262 A       | 6/1989  | Nishizawa et al.   |              | CN | 103958218 A       | 7/2014  |
| 4,862,486 A       | 8/1989  | Wing et al.        |              | CN | 104023997 A       | 9/2014  |
| 5,062,161 A       | 11/1991 | Sutton             |              | CN | 104343026 A       | 2/2015  |
| 5,135,039 A       | 8/1992  | Mizuta et al.      |              | CN | 107000483 A       | 8/2017  |
| 5,162,067 A       | 11/1992 | Miyawaki           |              | CN | 206646324 U       | 11/2017 |
| 5,213,652 A       | 5/1993  | Katoh et al.       |              | CN | 109952209 A       | 6/2019  |
| 5,223,060 A       | 6/1993  | Imamiya et al.     |              | DE | 102012214866 A1   | 2/2013  |
| 5,293,737 A       | 3/1994  | Kobayashi et al.   |              | EP | 0 125 518 A2      | 11/1984 |
| 5,295,346 A       | 3/1994  | Bundo et al.       |              | EP | 0376272 A1        | 7/1990  |
| 5,337,549 A       | 8/1994  | Kobayashi et al.   |              | EP | 1112868 A2        | 7/2001  |
| 5,502,960 A       | 4/1996  | Kobayashi et al.   |              | EP | 1 126 074 A2      | 8/2001  |
| 5,505,243 A       | 4/1996  | Imamiya et al.     |              | EP | 1 213 159 A2      | 6/2002  |
| 5,584,169 A       | 12/1996 | Ikehara            |              | EP | 1270270 A1        | 1/2003  |
| 5,802,830 A       | 9/1998  | Kawatani           |              | EP | 2218588 A1        | 8/2010  |
| 5,843,583 A       | 12/1998 | D'Haene et al.     |              | EP | 2261058 A1        | 12/2010 |
| 6,425,428 B1      | 7/2002  | Onuma et al.       |              | JP | 559677 A          | 3/1993  |
| 10,793,979 B2 *   | 10/2020 | Ridley .....       | D02G 1/0286  | JP | 7279071 A         | 10/1995 |
| 11,771,546 B2 *   | 10/2023 | Lima .....         | B01J 23/50   | JP | 2006183211 A      | 7/2006  |
|                   |         |                    | 623/14.13    | JP | 2007145125 A      | 6/2007  |
| 2001/0013385 A1   | 8/2001  | Ohya               |              | JP | 2009062655 A      | 3/2009  |
| 2002/0009608 A1   | 1/2002  | Nishikawa et al.   |              | JP | 2010-180483 A     | 8/2010  |
| 2002/0187345 A1   | 12/2002 | Andrews            |              | JP | 2010264878 A      | 11/2010 |
| 2003/0010418 A1   | 1/2003  | Miyazaki et al.    |              | KR | 101 194 309 B1    | 10/2012 |
| 2003/0046919 A1   | 3/2003  | Noferi             |              | WO | 2006010658 A1     | 2/2006  |
| 2003/0192157 A1   | 10/2003 | Andrews            |              | WO | WO 2007/128335 A1 | 11/2007 |
| 2005/0069685 A1   | 3/2005  | Andrews            |              | WO | 2012017399 A1     | 2/2012  |
| 2005/0183808 A1   | 8/2005  | Barguet et al.     |              | WO | WO 2012/055677 A2 | 5/2012  |
| 2005/0288775 A1 * | 12/2005 | Dong .....         | D02G 3/12    | WO | 2013098735 A1     | 7/2013  |
|                   |         |                    | 623/23.74    | WO | 2014083535 A2     | 6/2014  |
| 2006/0150378 A1   | 7/2006  | Andrews            |              | WO | 2015014639 A1     | 2/2015  |
| 2009/0176119 A1   | 7/2009  | Cristofani et al.  |              | WO | 2015097609 A1     | 7/2015  |
| 2010/0005774 A1   | 1/2010  | Fukuda             |              | WO | 2020021006 A1     | 1/2020  |
| 2010/0206450 A1   | 8/2010  | Fukumoto           |              |    |                   |         |
| 2010/0218872 A1   | 9/2010  | Ishizaka et al.    |              |    |                   |         |
| 2010/0300576 A1 * | 12/2010 | Liu .....          | D02G 3/406   |    |                   |         |
|                   |         |                    | 139/35       |    |                   |         |
| 2011/0099967 A1   | 5/2011  | Daghini et al.     |              |    |                   |         |
| 2011/0240626 A1 * | 10/2011 | Mullebrouck .....  | D02G 3/12    |    |                   |         |
|                   |         |                    | 219/260      |    |                   |         |
| 2011/0290398 A1   | 12/2011 | Kaoru              |              |    |                   |         |
| 2012/0267025 A1   | 10/2012 | Daghini et al.     |              |    |                   |         |
| 2013/0048185 A1   | 2/2013  | Harikae et al.     |              |    |                   |         |
| 2013/0118668 A1   | 5/2013  | Ascanelli et al.   |              |    |                   |         |
| 2014/0083590 A1   | 3/2014  | Ascanelli et al.   |              |    |                   |         |
| 2014/0338810 A1   | 11/2014 | Daghini et al.     |              |    |                   |         |
| 2015/0097662 A1   | 4/2015  | Yu et al.          |              |    |                   |         |
| 2015/0122395 A1   | 5/2015  | Misani et al.      |              |    |                   |         |
| 2016/0318343 A1   | 11/2016 | Daghini et al.     |              |    |                   |         |
| 2017/0027247 A1 * | 2/2017  | Lim .....          | A41D 31/0005 |    |                   |         |
| 2017/0313133 A1   | 11/2017 | Ascanelli et al.   |              |    |                   |         |
| 2018/0291535 A1 * | 10/2018 | Ridley .....       | D02G 3/406   |    |                   |         |
| 2018/0347078 A1 * | 12/2018 | Goenka .....       | D02G 3/286   |    |                   |         |
| 2018/0347080 A1 * | 12/2018 | Goenka .....       | D03D 15/54   |    |                   |         |
| 2019/0275835 A1   | 9/2019  | Rampana et al.     |              |    |                   |         |
| 2021/0000587 A1 * | 1/2021  | Lima .....         | D02G 3/448   |    |                   |         |
| 2021/0309050 A1   | 10/2021 | Cornille et al.    |              |    |                   |         |
| 2022/0371367 A1   | 11/2022 | Agresti et al.     |              |    |                   |         |
| 2023/0001741 A1   | 1/2023  | Agresti et al.     |              |    |                   |         |
| 2023/0366149 A1   | 11/2023 | Agresti et al.     |              |    |                   |         |

## FOREIGN PATENT DOCUMENTS

|    |           |         |
|----|-----------|---------|
| CN | 1280639 A | 1/2001  |
| CN | 1703551 A | 11/2005 |
| CN | 1708415 A | 12/2005 |
| CN | 1743188 A | 3/2006  |
| CN | 1965126 A | 5/2007  |

## OTHER PUBLICATIONS

International Search Report from the European Patent Office in corresponding International Application No. PCT/IB2020/062006 mailed Feb. 10, 2021.

Written Opinion of the International Searching Authority from the European Patent Office in corresponding International Application No. PCT/IB2020/062006 mailed Feb. 10, 2021.

Office Action issued by the European Patent Office on Oct. 4, 2024, in European Application No. 20 823 708.9 (7 pages).

Notification of the First Office Action issued by the China National Intellectual Property Administration on Jul. 18, 2023, in Chinese Application No. CN 202080085859.0 (10 pages) with English translation.

XP0558080809 Nokian Tyres PLC, "Reinforcing Materials in Rubber Products", Compound Development and Applications George Burrowes, The Goodyear Tire & Rubber Company, Mar. 1, 2015 (114 pages) [https://laroverket.com/wp-content/uploads/2015/03/reinforcing\\_materials.pdf](https://laroverket.com/wp-content/uploads/2015/03/reinforcing_materials.pdf).

Office Action issued by the European Patent Office on Dec. 7, 2023, in corresponding European Application No. 20 823 709.9 (7 pages). Third Party Observations issued by the European Patent Office on Oct. 6, 2023, in European Application No. 20823709.9 (12 pages). Notice of Allowance from Chinese Application No. 202080085859.0 issued May 2, 2024 (6 pages).

Third Party Observations issued by the European Patent Office on Apr. 10, 2024, in European Application No. 20823709.9 (7 pages). Office Action issued by the European Patent Office on Oct. 11, 2024, in European Application No. 20 823 709.9 (9 pages).

Notice of Allowance issued by the China National Intellectual Property Administration on May 23, 2024, in corresponding Application No. CN 202080085884.9 (5 pages).

Notification of the Second Office Action issued by the China National Intellectual Property Administration on Feb. 29, 2024, in corresponding Application No. CN 202080085884.9 (9 pages).

(56)

**References Cited**

OTHER PUBLICATIONS

Office Action issued by the European Patent Office on Jan. 18, 2024, in European Application No. EP 20 838 618.5 (6 pages).

Notification of the First Office Action issued by the China National Intellectual Property Administration on May 30, 2023, in corresponding Application No. CN 202080085884.9 (9 pages) and English translation.

International Search Report from the European Patent Office in corresponding International Application No. PCT/1B2020/062014 mailed Mar. 3, 2021.

Office Action issued by the European Patent Office on Nov. 15, 2024, in corresponding European Application No. 21 783 355.7 (6 pages).

Written Opinion of the International Searching Authority from the European Patent Office in corresponding International Application No. PCT/1B2020/062014 mailed Mar. 3, 2021.

International Search Report from the European Patent Office in corresponding International Application No. PCT/1B2020/062035 mailed Mar. 1, 2021.

Written Opinion of the International Searching Authority from the European Patent Office in corresponding International Application No. PCT/IB2020/062035 mailed Mar. 1, 2021.

International Search Report from the European Patent Office in corresponding International Application No. PCT/1B2021/058714 mailed Dec. 21, 2021.

Written Opinion of the International Searching Authority from the European Patent Office in corresponding International Application No. PCT/IB2021/058714 mailed Dec. 21, 2021.

\* cited by examiner



FIG. 1



FIG. 2



FIG. 3



FIG. 3a



FIG. 4





FIG. 6



FIG. 7



FIG. 8



FIG. 9



FIG. 10



FIG. 11



FIG. 12



FIG. 13



FIG. 14



FIG. 15



FIG. 16



FIG. 17





FIG. 19



FIG. 20



FIG. 21

FIG. 22



**PROCESS AND APPARATUS FOR  
MANUFACTURING A METALLIC  
REINFORCING CORD FOR TYRES FOR  
VEHICLE WHEELS**

This application is a national stage filing under 35 U.S.C. § 371 of International Application No. PCT/IB2021/062006, filed on Dec. 16, 2020, and claims priority to Italian Application No. 102019000024280, filed Dec. 17, 2019; the disclosure of each of these applications are incorporated herein by reference in their entirety.

**DESCRIPTION**

The present invention relates to a process and an apparatus for manufacturing a metallic reinforcing cord for tyres for vehicle wheels.

**PRIOR ART**

Metallic reinforcing cords for tyres for vehicle wheels and processes and apparatuses for manufacturing metallic reinforcing cords are described in US2003046919 and in WO2007128335 to the Applicant and in WO2012055677.

**SUMMARY OF THE INVENTION**

Hereinafter, when reference is made to any range of values comprised between a minimum value and a maximum value, the aforementioned minimum and maximum values are included in the aforementioned range, unless expressly stated to the contrary.

Moreover, all of the ranges include any combination of the maximum and minimum values described and include any intermediate range, even if not expressly specifically described.

Any numerical value is considered to be preceded by the term "about" to also indicate any numerical value that differs slightly from the one described, for example to take into account the typical dimensional tolerances in the field of reference.

Hereinafter the following definitions apply.

The term "equatorial plane" of the tyre is used to indicate a plane perpendicular to the rotation axis of the tyre and that divides the tyre into two symmetrically equal parts.

The terms "radial" and "axial" and the expressions "radially inner/outer" and "axially inner/outer" are used with reference, respectively, to a direction substantially parallel to the equatorial plane of the tyre and to a direction substantially perpendicular to the equatorial plane of the tyre, i.e. to a direction substantially perpendicular to the rotation axis of the tyre and to a direction substantially parallel to the rotation axis of the tyre, respectively.

The terms "circumferential" and "circumferentially" are used with reference to the direction of annular extension of the tyre, i.e. to the rolling direction of the tyre, which corresponds to a direction lying on a plane coinciding with or substantially parallel to the equatorial plane of the tyre.

The term "substantially axial direction" is used to indicate a direction inclined, with respect to the equatorial plane of the tyre, by an angle comprised between 70° and 90°.

The term "substantially circumferential direction" is used to indicate a direction oriented, with respect to the equatorial plane of the tyre, at an angle comprised between 0° and 10°.

The expressions "upstream" and "downstream" are used with reference to a predetermined direction and to a predetermined reference. Therefore, assuming for example a

direction from left to right and a reference taken along said direction, a position "downstream" with respect to the reference indicates a position to the right of said reference and a position "upstream" with respect to the reference indicates a position to the left of said reference.

The term "elastomeric material" is used to indicate a material comprising a vulcanizable natural or synthetic polymer and a reinforcing filler, wherein such a material, at room temperature and after having been subjected to vulcanization, can undergo deformations caused by a force and is capable of quickly and energetically recovering the substantially original shape and size after the elimination of the deforming force (according to the definitions of ASTM D1566-11 Standard Terminology Relating To Rubber).

The term "metallic reinforcing cord" is used to indicate an element consisting of one or more elongated elements (also called "wires") made of a metallic material and possibly coated by, or incorporated in, a matrix of elastomeric material.

The term "hybrid reinforcing cord" is used to indicate a reinforcing cord comprising at least one metallic wire twisted together with at least one textile yarn. Hereinafter, reference is made to hybrid reinforcing cords reference to refer, in particular, to reinforcing cords comprising textile yarns having low modulus, like for example nylon yarns.

The term "mixed textile reinforcing cord" is used to indicate a reinforcing cord comprising at least one textile yarn having a low modulus, like for example a nylon yarn, twisted together with at least one textile yarn having a high modulus, like for example an aramid yarn.

The term "yarn" is used to indicate an elongated element consisting of the aggregation of a plurality of textile filaments or fibers.

The yarns can have one or more "ends", where the term "end" is used to indicate a bundle of filaments twisted together. Preferably, a single end or at least two ends twisted together are provided.

The yarn can be identified with a symbol that represents the textile material, the linear density of the fiber used and the number of ends that form the yarn. For example, an aramid yarn (aromatic polyamide) identified as Ar1672 indicates a textile yarn comprising Aramid fibers with a linear density of 1670 dtex, formed by two ends twisted together.

The term "strand" is used to indicate the union of at least two wires or yarns, or of at least one wire and at least one yarn, to constitute an elongated element intended to be twisted together with at least one other elongated element to form at least one part of a reinforcing cord.

The term "diameter" of a reinforcing cord, or of a wire, is used to indicate the diameter measured as prescribed by the method BISFA E10 (The International Bureau For The Standardization Of Man-Made Fibres, Internationally Agreed Methods For Testing Steel Tyre Cords, 1995 edition).

In the case of yarns, the term "diameter" is used to indicate the diameter of an ideal circumference that circumscribes all of the filaments that define the yarn. The diameter of a yarn increases as the number of filaments and/or ends of the yarn increases.

The term "thread count" of a layer is used to indicate the number of reinforcing cords per unit length provided in such a layer. The thread count can be measured in cords/dm (number of cords per decimeter).

The term "linear density" or "count" of a cord or yarn is used to indicate the weight of the cord or yarn per unit length. The linear density can be measured in dtex (grams per 10 km length).

The term "modulus" is used to indicate the ratio between load (or force) and elongation measured at any point of a load-elongation curve according to the BISFA standard. Such a curve is traced by calculating the first derivative of the load-elongation function that defines the aforementioned curve, normalized to the linear density expressed in Tex. The modulus is therefore expressed in cN/Tex. In a load-elongation graph, the modulus is identified by the slope of the aforementioned curve with respect to horizontal axis.

The term "initial modulus" is used to indicate the modulus calculated at the origin point of the load-elongation curve, i.e. for an elongation equal to zero.

The term "high modulus" is used to indicate an initial modulus equal to or greater than 3000 cN/Tex. The term "low modulus" is used to indicate an initial modulus lower than 3000 cN/Tex.

For the measurement of the linear density and of the modulus reference is made to flat wires/yarns, without twists applied in the testing phase or twisting phase, according to the tests regulated by BISFA.

The term "breaking load" and "elongation at break" of a reinforcing cord are used to indicate the load and the percentage elongation, respectively, at which the reinforcing cord breaks, evaluated with the method BISFA E6 (The International Bureau For The Standardization Of Man-Made Fibres, Internationally Agreed Methods For Testing Steel Tyre Cords, 1995 edition).

The term "part load elongation" of a reinforcing cord is used to indicate the difference between the percentage elongation obtained by subjecting the reinforcing cord to a traction of 50 N and the percentage elongation obtained by subjecting the reinforcing cord to a traction of 2.5 N. The part load elongation is evaluated with the method BISFA E7 (The International Bureau For The Standardization Of Man-Made Fibres, Internationally Agreed Methods For Testing Steel Tyre Cords, 1995 edition).

The term "rigidity" of a reinforcing cord is used to indicate the resistant moment to bending with a predetermined angle (normally 15°) evaluated with the method BISFA E8 (The International Bureau For The Standardization Of Man-Made Fibres, Internationally Agreed Methods For Testing Steel Tyre Cords, 1995 edition).

The term "metallic reinforcing cord having a high elongation", or "HE metallic reinforcing cord", is used to indicate a reinforcing cord that has:

a) an elongation at break equal to at least 3.5% and, preferably

b) a part load elongation comprised between 1% and 3%.

Feature "a" cited above is calculated with the method BISFA E6 (The International Bureau For The Standardization Of Man-Made Fibres, Internationally Agreed Methods For Testing Steel Tyre Cords, 1995 edition). Feature "b" cited above is calculated with the method BISFA E7 (The International Bureau For The Standardization Of Man-Made Fibres, Internationally Agreed Methods For Testing Steel Tyre Cords, 1995 edition).

The term "wire made of NT steel" (Normal Tensile Steel) is used to indicate a wire made of carbon steel having a tensile strength of 2800±200 MPa, for example having a tensile strength of at least 2700 MPa for a wire diameter of 0.28 mm.

The term "wire made of HT steel" (High Tensile Steel) is used to indicate a wire made of carbon steel having a tensile

strength of 3200±200 MPa, for example a tensile strength of at least 3100 MPa for a wire diameter of 0.28 mm.

The term "wire made of ST steel" (Super Tensile Steel) is used to indicate a wire made of carbon steel having a tensile strength of 3500±200 MPa, for example a tensile strength of at least 3400 MPa for a wire diameter of 0.28 mm.

The term "wire made of UT steel" (Ultra Tensile Steel) is used to indicate a wire made of carbon steel having a tensile strength of 3900±200 MPa, for example a tensile strength of at least 3800 MPa for a wire diameter of 0.28 mm.

The tolerances ±200 MPa are indicated to comprise, for each class of steel, the minimum and maximum tensile strength values due to the various wire diameters (typically the tensile strength value is inversely proportional to the diameter of the wire), for example for wire diameters comprised between 0.12 mm and 0.40 mm.

The term "mechanical behavior" of a reinforcing cord is used to indicate the reaction offered by the reinforcing cord when subjected to a load (or force). In the case of a traction load, such a load results in an elongation that is variable depending on the amount of the load according to a function identified by a particular load-elongation curve. The mechanical behavior depends on the material of the wire(s) and/or yarn(s) used, on the number of such wires/yarns, on their diameter or linear density and on the possible twisting pitch.

The expression "unravelling" of a reinforcing cord is used to indicate the tendency of single wires and/or yarns of the reinforcing cord not to remain stably woven when the reinforcing cord is subjected to cutting with a cutter. The unravelling is evaluated with the method BISFA E3 (The International Bureau For The Standardization Of Man-Made Fibres, Internationally Agreed Methods For Testing Steel Tyre Cords, 1995 edition).

The term "high performance tyres" is used to indicate tyres which are typically intended to be used in wheels of high and ultra-high-performance automobiles. Such tyres are commonly defined as "HP" or "UHP" and allow speeds of over 200 km/h, up to more than 300 km/h, to be reached.

Examples of such tyres are those belonging to classes "T", "U", "H", "V", "Z", "W", "Y", according to the E.T.R.T.O.—(European Tyre and Rim Technical Organisation) standard and racing tyres, in particular for high piston displacement four-wheeled vehicles. Typically, tyres belonging to such classes have section width equal to or greater than 185 mm, preferably comprised between 195 mm and 385 mm, more preferably comprised between 195 mm and 355 mm. Such tyres are preferably mounted on rims having fitting diameters equal to or greater than 13 inches, preferably not greater than 24 inches, more preferably comprised between 16 inches and 23 inches. Such tyres can also be used in vehicles different from the aforementioned automobiles, for example in high-performance sports motorcycles, i.e. motorcycles capable of reaching speeds even over 270 km/h. Such motorcycles are those that belong to the category typically identified with the following classifications: hypersport, supersport, sport touring, and for lower speed rating: scooter, road enduro and custom.

The term "tyre for motorcycle wheels" is used to indicate a tyre having a high curvature ratio (typically more than 0.200), capable of reaching high camber angles when the motorcycle is cornering.

The term "tyre for heavy and/or light load vehicle wheels", is used to indicate a tyre intended to be used in a vehicle belonging to categories M2, M3, N2, N3 and 02-04, according to the "ECE Consolidated Resolution of the Construction of vehicles (R.E. 3), Annex 7, Classification

and definition of power driven vehicles and trailers", or to categories M3, N2, N3, O3, O4 according to the "ETRTO Engineering design information" (2010 edition), "General Information" section, pages G15 and G16, chapter "International codes for wheeled vehicle classification as UN/ECE 29/78 and Directive 2003/37".

Hereinafter, when reference is made to automobile tyres both tyres for cars, like for example the high performance tyres defined above, and tyres for light load vehicles, for example trucks, vans, campervans, pick-up trucks, typically with a total mass at full load equal to or lower than 3500 Kg, are intended.

The term "radial carcass structure" is used to indicate a carcass structure comprising a plurality of reinforcing cords, each of which being oriented along a substantially axial direction. Such reinforcing cords can be incorporated in a single carcass layer or in a plurality of carcass layers (preferably two) radially juxtaposed over one another.

The term "crossed belt structure" is used to indicate a belt structure comprising a first belt layer including reinforcing cords substantially parallel to one another and inclined with respect to the equatorial plane of the tyre by a predetermined angle and at least one second belt layer arranged in a radially outer position with respect to the first belt layer and including reinforcing cords substantially parallel to one another and oriented with an inclination opposite to the one of the cords of the first layer with respect to the equatorial plane of the tyre.

The term "zero degrees belt layer" is used to indicate a reinforcing layer comprising at least one reinforcing cord wound on the belt structure according to a substantially circumferential winding direction.

The term "stoneguard layer" is used to indicate a layer specially provided, typically in tyres for heavy and/or light load vehicle wheels, in a radially outer position with respect to the belt structure to protect the latter (and the underlying carcass structure) from undesired objects or external elements (for example stones and/or gravel and/or water and/or moisture) and/or from rough parts which are on a road surface. Such a stoneguard layer comprises a plurality of cords parallel to one another and extending according to a substantially circumferential direction.

In order to keep down the emissions of CO<sub>2</sub> into the atmosphere, the Applicant has been producing for many years tyres for automobile, motorcycle and heavy and/or light load vehicle wheels having a low rolling resistance. Such tyres comprise, in the respective crossed belt structures, and/or in the bead reinforcing structures indicated below with "chafer" and "flipper" and/or, in the specific case of tyres for heavy and/or light load vehicle wheels, in the stoneguard layer, metallic reinforcing cords comprising particularly light steel wires, for example having a diameter equal to 0.22 mm, 0.20 mm or 0.175 mm.

The choice of the Applicant to use in the aforementioned structural components of the tyre reinforcing cords comprising only steel wires derives from the fact that the steel wires, having a high rigidity and an excellent resistance to fatigue, are capable of providing the reinforcing cord, and thus the aforementioned structural components of the tyre, with a high resistance to the high compressive or bending stresses to which such structural components are typically subjected during travel of the vehicle on which the tyre is mounted. Moreover, thanks to the high heat conduction capability of steel, the steel wires have high thermal stability, providing the reinforcing cord with a stable mechanical behavior even in extreme conditions of use, like those typical of high performance tyres.

The Applicant has also observed that steel ensures good adhesion of the reinforcing cord to the surrounding elastomeric material, with consequent advantages in terms of quality of the tyre.

However, the Applicant observed that in order to avoid risks of corrosion of the steel in the case of leakage of water inside the tyre and, at the same time, to maximize the adhesion between steel and elastomeric material, it is advisable to ensure that, at each cross section of the reinforcing cord and, therefore, along the entire longitudinal extension of the reinforcing cord, the elastomeric material surrounds as completely as possible each steel wire. In the case of reinforcing cords comprising a plurality of steel wires twisted together, it is also advisable for the elastomeric material to penetrate as much as possible into the space defined between the aforementioned wires. This is in order to avoid having zones of possible mutual contact of the steel wires, which would actually constitute zones of possible formation of cracks due to fatigue from fretting, at the expense of the structural integrity of the tyre.

The Applicant has also observed that steel wires, having a low part load elongation, are not suitable for being used in those structural components of the tyre where a high part load elongation is desired, like for example in the zero degrees belt layers. In such structural components it is deemed preferable to use textile reinforcing cords having a low modulus, like for example reinforcing cords made of nylon or, in the cases in which a high rigidity is also required at high loads (and thus a high modulus at high loads), mixed textile reinforcing cords or hybrid reinforcing cords.

With particular reference to mixed textile reinforcing cords and hybrid reinforcing cords, they make it possible to obtain the desired part load elongation and the desired rigidity thanks to their characteristic "double modulus" mechanical behavior obtained through the use of a material having a low modulus and a material having a high modulus. At low loads, the mechanical behavior of the reinforcing cord is mainly dictated by the reaction offered by the material having low modulus, whereas at high loads the mechanical behavior of the reinforcing cord is mainly dictated by the reaction offered by the material having high modulus. Such types of reinforcing cords therefore have a mechanical behavior that translates, in a load-elongation graph, by a curve defined by two segments separated by a joining knee, wherein the segment on the left of the knee (indicative of the part load elongations) has a much lower inclination with respect to the horizontal axis than that of the segment on the right of the knee (indicative of the rigidity).

The Applicant has however observed that the textile and hybrid reinforcing cords, unlike the metallic ones, do not allow adequate adhesion of the surrounding elastomeric material. Therefore, it is necessary to coat them with adhesive substances or subject them to specific chemical or physical adhesive-fixing treatments.

The Applicant has thought that it would be desirable to also use metallic reinforcing cords in those structural components of the tyre where textile or hybrid reinforcing cords are currently used, so as to obtain also in such structural components an adequate adhesion between reinforcing cord and surrounding elastomeric material with no need to apply an adhesive coating to the reinforcing cord or to subject it to adhesion-fixing treatments.

The Applicant has found that it is possible to satisfy this desire by providing metallic reinforcing cords having a helical geometry.

The Applicant has indeed realized that such a particular geometry allows the reinforcing cord to have a mechanical

behavior at low loads that is comparable to that of textile reinforcing cords having a low modulus (thus obtaining a high part load elongation) and a mechanical behavior at high loads that is comparable to that of metallic reinforcing cords (thus obtaining a high rigidity). The high part load elongation is a consequence of the stretching of the helix defining the metallic reinforcing cord (the reinforcing cord in this case behaves like a spring), whereas the high rigidity at high loads is a consequence of the high elastic modulus which is typical of the metallic material.

In practice, due to the aforementioned helical geometry the metallic reinforcing cords can have a "double modulus" mechanical behavior which is comparable to the mechanical behavior which is typical of mixed and hybrid textile reinforcing cords. It is therefore possible to use the aforementioned metallic reinforcing cords in all those structural components of the tyre where hybrid and mixed textile reinforcing cords are typically used, obtaining all of the abovementioned advantages linked to the use of metallic reinforcing cords (in particular: fatigue resistance, thermal stability and adhesion).

The Applicant has found that the aforementioned helical geometry allows an improvement of the adhesion between reinforcing cord and surrounding elastomeric material also in the case in which the metallic reinforcing cord comprises a single metallic wire. This is due to a better mechanical adhesion of the elastomeric material on a helical wire with respect to a substantially straight wire.

The Applicant has also found that, in the case in which the metallic reinforcing cord comprises a plurality of steel wires twisted together, the helical geometry makes it possible to obtain, in addition to the desired improvement in terms of adhesion, a better penetration of the elastomeric material inside the metallic reinforcing cord, with consequent advantages in terms of resistance to corrosion and to fatigue from fretting.

The Applicant is also convinced that the helical geometry, providing the reinforcing cords with the capability of extending longitudinally when subjected to a load, allows the metallic reinforcing cords used in the crossed belt structures to maintain their design angle of inclination during the tyre shaping process.

The present invention therefore relates, in a first aspect thereof, to a process for manufacturing a metallic reinforcing cord for tyres for vehicle wheels.

Preferably, at least one elongated element comprising at least one metallic wire twisted together with at least one textile yarn is provided.

Preferably, said at least one textile yarn is removed from said at least one elongated element to form a metallic reinforcing cord in which said at least one metallic wire extends along a helical path.

In a second aspect thereof, the invention relates to an apparatus for manufacturing a metallic reinforcing cord for tyres for vehicle wheels from at least one elongated element comprising at least one metallic wire twisted together with at least one textile yarn.

Preferably, a removal device is provided, the removal device being configured to remove said at least one textile yarn from said at least one elongated element to form a metallic reinforcing cord in which said at least one metallic wire extends along a helical path.

Such an apparatus makes it possible to obtain a metallic reinforcing cord in accordance with the first aspect of the invention.

In the present invention, the textile yarn is therefore a "throwaway" element, i.e. an element only used to provide

said at least one metallic wire with a helical geometry. The textile yarn is thus intended to be removed, so as to obtain a metallic reinforcing cord consisting only of said at least one metallic wire and therefore also having a helical geometry. Such a metallic reinforcing cord has, in addition to those advantageous features which are typical of the metallic reinforcing cords (rigidity at high loads, fatigue resistance, thermal stability and adhesion to elastomeric material), a high penetration of the elastomeric material inside it (in the 10 case in which the metallic reinforcing cord comprises a plurality of metallic wires) and a high part load elongation.

The particular helical geometry of the metallic reinforcing cord of the invention can be selected, depending on the 15 particular application, by changing one or more among the twisting pitch with which said at least one metallic wire is 20 twisted about said at least one textile yarn, the diameter of said at least one metallic wire, the number of metallic wires, the diameter of said at least one textile yarn (i.e. the number of filaments and/or ends of the textile yarn), the number of 25 textile yarns.

Depending on the particular helical geometry which is 30 selected the reinforcing cord can be more suitable for being used in some structural components of the tyre with respect to other structural components of the tyre. For example, it is 35 possible to foresee a helical geometry adapted to maximize the rigidity, and/or the breaking load and/or, in the case in which the reinforcing cord comprises a plurality of metallic wires, the penetration of the elastomeric material inside the 40 space defined between the various metallic wires, or a different helical geometry adapted to maximize the part load elongation and/or the elongation at break.

According to the Applicant, it is preferable to maximize the rigidity and/or the breaking load and/or the penetration when using the metallic reinforcing cord in the crossed belt 45 structures of the tyres for automobile or heavy and/or light load vehicle wheels, or in the reinforcing structures of the bead, indicated below with "chafer" and "flipper", of tyres for car, motorcycle or heavy and/or light load vehicle 50 wheels, or in the stonguard layer of the latter, or in the carcass structures of tyres for motorcycle or heavy and/or light load vehicle wheels, whereas it is preferable to maximize the part load elongation and/or the elongation at break when using the metallic reinforcing cord in the zero degrees belt layers of tyres for car, heavy and/or light load vehicle 55 and motorcycle wheels.

The Applicant believes that it may be advantageous to maximize the part load elongation also in the carcass structures of tyres, in order to increase the penetration of the elastomeric material inside the reinforcing cords.

The Applicant believes that, for example:

in order to maximize the rigidity and/or the breaking load it is possible to increase the number and/or the diameter of the metallic wires or decrease the diameter of said at least one textile yarn (i.e. the number of filament and/or ends of the textile yarn), while keeping the other parameters unchanged;

in order to maximize the penetration it is possible to increase the twisting pitch of said at least one metallic wire about said at least one textile yarn, or the diameter of said at least one textile yarn (i.e. the number of filaments and/or ends of the textile yarn), while keeping the other parameters unchanged;

in order to maximize the part load elongation and/or the elongation at break it is possible to increase the diameter of said at least one textile yarn (i.e. the number of filaments and/or ends of the textile yarn) or to reduce the twisting pitch of said at least one metallic wire

about said at least one textile yarn, while keeping the other parameters unchanged.

In at least one of the aforementioned aspects, the present invention can have at least one of the preferred features described hereinafter. Such features can therefore be provided singularly or in combination with each other, except when expressly stated otherwise.

The elongated element, once obtained, can be wound in a service reel, from which it is subsequently taken to remove the textile yarn and, therefore, to manufacture the metallic reinforcing cord.

Alternatively, the elongated element can be fed continuously along a predetermined feeding direction to remove the textile yarn and, therefore, to manufacture the metallic reinforcing cord. In this last case, the removal of the textile yarn from the elongated element is carried while obtaining said at least one elongated element and, therefore, while manufacturing the metallic reinforcing cord.

In both of the cases discussed above, said at least one elongated element is obtained by feeding said at least one metallic wire and said at least one textile yarn to a twisting device.

Preferably, said at least one textile yarn is made of a water-soluble material, more preferably of a water-soluble synthetic polymeric material, even more preferably of a polyvinyl alcohol (PVA). Such a material is non-toxic, colorless and odorless, and therefore its use does not cause any risk to the workers that handle it or that are in the vicinity of it.

Preferably, removing said at least one textile yarn comprises feeding a hot water jet against said at least one elongated element.

Preferably, after removing said at least one textile yarn, said metallic reinforcing cord is dried.

Preferably, said metallic reinforcing cord, possibly after being dried, is wound on a collection reel from which it is then taken to build the tyre or structural components thereof.

As an alternative to the removal through a hot water jet it is possible to provide for a mechanical removal through a device configured to unwind the textile yarn from the metallic wire(s), or a removal through steam, or a removal through thermal disintegration of the textile yarn with subsequent removal of the fragments of the latter through blowing of air or soaking in water.

In preferred embodiments of the invention, said at least one elongated element comprises at least two metallic wires twisted together with said at least one textile yarn. Consequently, the metallic reinforcing cord consists of a plurality of metallic wires twisted together, each metallic wire having a helical geometry.

Said at least two metallic wires can be twisted together with said at least one textile yarn with the same twisting pitch and same twisting direction, or with the same twisting pitch and opposite twisting directions, or with different twisting pitch and the same twisting direction, or with different twisting pitches and opposite twisting directions.

Said at least two metallic wires may or may not have the same diameter.

Preferably, said at least two metallic wires are made of steel. Such steel wires may or may not have the same carbon content.

A metallic reinforcing cord comprising a plurality of metallic wires is particularly suitable for allowing an adequate penetration of the elastomeric material inside the space defined between said metallic wires, thus protecting the reinforcing cord from possible corrosion phenomena due to a leakage of water inside the tyre, avoiding undesired

fretting phenomena and maximizing the adhesion between reinforcing cord and elastomeric material. In fact, the elastomeric material takes up the free space left by the textile yarn after the latter is removed.

The elastomeric material arranged between the metallic wires also tends to behave like a structural component of the reinforcing cord and thus it also gives a contribution in terms of rigidity.

By increasing the diameter, or the linear density, of the 10 textile yarn it is possible to increase the amount of elastomeric material incorporated between the metallic wires of the reinforcing cord and more evenly distribute the steel wires in a piece of structural component having a predetermined thickness, achieving an increased rigidity of such a 15 structural component and a better transmission of the stresses to which such a structural component is subjected during use of the tyre, to the benefit of the responsiveness.

A further advantageous effect linked to the greater uniformity of distribution of the metallic wires in the piece of 20 structural component is that it is possible to increase the winding pitch of the helix with no risk that unravelling occurs. This allows an increase in the amount of metallic 25 reinforcing cord produced in a predetermined time period to be achieved (hereinafter such a feature is also indicated as "machine output"), with consequent economic and production advantages.

Assuming, as an example, that the elongated element (comprising one or more strands of metallic wires twisted together with one or more textile yarns) and the metallic 30 reinforcing cord (comprising one or more strands of metallic wires twisted together) have substantially circular cross sections, it is possible to make the elongated element so that the textile yarn is arranged only between substantially circumferentially opposite metallic wires or only between 35 substantially circumferentially adjacent metallic wires or both between substantially circumferentially opposite metallic wires and between substantially circumferentially adjacent metallic wires. In this case, the space provided in the reinforcing cord after the removal of the textile yarn and 40 intended to be occupied by the elastomeric material will be either only the inner space defined between the various wires, or only the outer space defined between circumferentially adjacent wires or both the inner space defined between the various wires and the outer space defined 45 between circumferentially adjacent wires. In the case the elongated element comprises a plurality of strands, each strand comprising a plurality of metallic wires twisted together with a respective textile yarn, the textile yarn can be removed from only some of the aforementioned strands or 50 from all of the aforementioned strands.

In some preferred embodiments thereof, said metallic reinforcing cord comprises a plurality of cross sections in which said at least two metallic wires are in a condition of substantial mutual contact.

Preferably, said metallic reinforcing cord also comprises other cross sections in which said at least two metallic wires are spaced from one another.

It is however possible to actuate solutions suitable for ensuring that in all of the cross sections of the reinforcing cord said at least two metallic wires are spaced from one another.

Such solutions consist, preferably, in suitably deforming (or preforming or crimping) the metallic reinforcing cord until all of the metallic wires are spaced apart from one another along the entire longitudinal extension of the reinforcing cord. Such a deformation (or preforming or crimping) can be obtained by providing the metallic reinforcing

## 11

cord with very high curvatures through passage of the reinforcing cord over a plurality of cylinders having a reduced diameter (for example comprised between 1 and 5 mm) with a predetermined pull.

In some embodiments, therefore, deforming the metallic reinforcing cord comprises pulling said metallic reinforcing cord by a traction force that is constant or variable over time. It is possible in this way to adjust as desired the relative spacing of the various metallic wires and, therefore, their distribution in a predetermined piece of structural component of the tyre.

As the spacing between the various metallic wires changes, both the penetration of the elastomeric material in the metallic reinforcing cord and the rigidity of the metallic reinforcing cord change.

In accordance with the present invention, the removal device is arranged, with respect to a feeding direction of said at least one elongated element, downstream of a service reel configured to collect said at least one elongated element or, in the case in which the removal of said at least one textile yarn is carried out while said at least one elongated element is obtained, downstream of a twisting device configured to twist together said at least one metallic wire and said at least one textile yarn thus obtaining said at least one elongated element.

The aforementioned service reel, when provided, is arranged downstream of a twisting device configured to twist together said at least one metallic wire and said at least one textile yarn thus obtaining said at least one elongated element.

Preferably, a collection reel configured to collect said metallic reinforcing cord is provided downstream of said removal device.

Preferably, the removal device comprises a hot water jet feeding device.

Preferably, a drying device is provided downstream of said feeding device.

As already stated, it is possible to foresee removal systems of the textile yarn different from those based on the feeding of a hot water jet.

The metallic reinforcing cord obtained through the present invention can have a part load elongation greater than 1%, preferably greater than 2%, even greater than 3%, even greater than or equal to 3.5%, preferably even greater than or equal to 4%, even more preferably even greater than or equal to 5%.

Said metallic reinforcing cord can have a twisting pitch greater than or equal to 2 mm, preferably greater than or equal to 3 mm, even more preferably greater than or equal to 4 mm, even more preferably greater than or equal to 5 mm.

Said metallic reinforcing cord can have an elongation at break greater than 5%, preferably up to 20%, more preferably up to 15%.

## DESCRIPTION OF THE FIGURES

Further features and advantages of the present invention will become clearer from the following detailed description of a preferred embodiment thereof, made with reference to the attached drawings.

In such drawings:

FIG. 1 is a schematic partial half cross-section view of a portion of a possible embodiment of a tyre in which a metallic reinforcing cord in accordance with the present invention can be used;

## 12

FIG. 2 is a photo of a segment of a first embodiment of a metallic reinforcing cord in accordance with the present invention;

FIG. 3 is a photo of a textile yarn used to manufacture the metallic reinforcing cord of FIG. 2;

FIG. 3a is a photo of an elongated element used to manufacture the metallic reinforcing cord of FIG. 2 through the textile yarn of FIG. 3;

FIG. 4 is a schematic view of a first embodiment of an apparatus for manufacturing the metallic reinforcing cord in accordance with the present invention, such an apparatus carrying out a continuous process;

FIGS. 5a and 5b show a second embodiment of an apparatus for manufacturing the metallic reinforcing cord in accordance with the present invention, such an apparatus carrying out a discontinuous process;

FIGS. 6-10 show some load-elongation graphs of conventional cords and of metallic reinforcing cords made in accordance with the present invention;

FIGS. 11-20 show various examples of metallic reinforcing cords made in accordance with the present invention and of conventional metallic reinforcing cords; some cross sections of each of the aforementioned reinforcing cords in a respective piece of elastomeric material are also illustrated;

FIGS. 21 and 22 show respective segments of further embodiments of metallic reinforcing cords made in accordance with the present invention.

DETAILED DESCRIPTION OF EMBODIMENTS  
OF THE INVENTION

For the sake of simplicity, FIG. 1 shows only part of an embodiment of a tyre 100 produced with the method and the apparatus of the present invention, the remaining part, which is not shown, being substantially identical and being arranged symmetrically with respect to the equatorial plane M-M of the tyre.

The tyre 100 shown in FIG. 1 is, in particular, a tyre for four-wheeled vehicles.

Preferably, the tyre 100 is a HP or UHP tyre for sports and/or high or ultra-high-performance automobiles.

In FIG. 1 "a" indicates an axial direction, "c" indicates a radial direction, "M-M" indicates the equatorial plane of the tyre 100 and "R-R" indicates the rotation axis of the tyre 100.

The tyre 100 comprises at least one support structure 100a and, in a radially outer position with respect to the support structure 100a, a tread band 109 made of elastomeric material.

The support structure 100a comprises a carcass structure 101, which comprises at least one carcass layer 111.

Hereinafter, for the sake of simplicity of description, reference will be made to an embodiment of the tyre 100 comprising a single carcass layer 111, being nevertheless understood that what is described has analogous application in tyres comprising more than one carcass layer.

The carcass layer 111 has axially opposite end edges engaged with respective annular anchoring structures 102, called bead cores, possibly associated with an elastomeric filler 104. The zone of the tyre 100 comprising the bead core 102 and the possible elastomeric filler 104 forms an annular reinforcing structure 103 called "bead structure" and intended to allow the anchoring of the tyre 100 on a corresponding mounting rim, not shown.

The carcass layer 111 comprises a plurality of reinforcing cords 10' coated with an elastomeric material or incorporated in a matrix of cross-linked elastomeric material.

## 13

The carcass structure 101 is of the radial type, i.e. the reinforcing cords 10<sup>1</sup> are on planes comprising the rotation axis R-R of the tyre 100 and substantially perpendicular to the equatorial plane M-M of the tyre 100.

Each annular reinforcing structure 103 is associated with the carcass structure 101 by folding back (or turning) the opposite end edges of the at least one carcass layer 111 about the bead core 102 and the possible elastomeric filler 104, so as to form the so-called turnings 101a of the carcass structure 101.

In an embodiment, the coupling between carcass structure 101 and annular reinforcing structure 103 can be made through a second carcass layer (not shown in FIG. 1) which is applied in a radially outer position with respect to the carcass layer 111.

An anti-abrasion strip 105 is arranged at each annular reinforcing structure 103 so as to wrap around the annular reinforcing structure 103 along the axially inner, axially outer and radially inner zones of the annular reinforcing structure 103, thus being arranged between the latter and the rim of the wheel when the tyre 100 is mounted on the rim. However, embodiments wherein such an anti-abrasion strip 105 is not provided are foreseen.

The support structure 100a comprises, in a radially outer position with respect to the carcass structure 101, a crossed belt structure 106 comprising at least two belt layers 106a, 106b arranged in radial juxtaposition with respect to one another.

The belt layers 106a, 106b respectively comprise a plurality of reinforcing cords 10a, 10b. Such reinforcing cords 10a, 10b have an inclined orientation with respect to the circumferential direction of the tyre 100, or to the equatorial plane M-M of the tyre 100, by an angle comprised between 15° and 45°, preferably between 20° and 40°. For example, such an angle is equal to 30°.

The support structure 100a can also comprise a further belt layer (not shown) arranged between the carcass structure 101 and the radially inner belt layer of the aforementioned belt layers 106a, 106b and comprising a plurality of reinforcing cords having an inclined orientation with respect to the circumferential direction of the tyre 100, or to the equatorial plane M-M of the tyre 100, by an angle equal to 90°.

The support structure 100a can also comprise a further belt layer (not shown) arranged in a radially outer position with respect to the radially outer belt layer of the aforementioned belt layers 106a, 106b and comprising a plurality of reinforcing cords having an inclined orientation with respect to the circumferential direction of the tyre 100, or to the equatorial plane M-M of the tyre 100, by an angle comprised between 20° and 70°.

The reinforcing cords 10a, 10b of a belt layer 106a, 106b are parallel to one another and have a crossed orientation with respect to the reinforcing cords of the other belt layer 106b, 106a.

In ultra-high-performance tyres, the belt structure 106 can be a turned crossed belt structure. Such a belt structure is made by arranging at least one belt layer on a support element and turning the opposite lateral end edges of said at least one belt layer. Preferably, a first belt layer is initially deposited on the support element, then the support element radially expands, then a second belt layer is deposited on the first belt layer and finally the opposite axial end edges of the first belt layer are turned on the second belt layer to at least partially cover the second belt layer, which is the radially outermost layer. In some cases, it is possible to deposit a third belt layer on the second belt layer. Advantageously, the

## 14

turning of the axially opposite end edges of a belt layer on a radially outer belt layer imparts greater reactivity and responsiveness of the tyre when entering a bend.

The support structure 100a comprises, in a radially outer position with respect to the crossed belt structure 106, at least one zero degrees belt layer 106c, commonly known as "zero degrees belt". It comprises reinforcing cords 10c oriented along a substantially circumferential direction. Such reinforcing cords 10c thus form an angle of a few degrees (typically lower than 10°, for example comprised between 0° and) 6° with respect to the equatorial plane M-M of the tyre 100.

The tread band 109 is applied in a radially outer position with respect to the zero degrees belt layer 106c, like other semi-finished products which constitute the tyre 100.

Respective sidewalls 108 made of elastomeric material are also applied on the opposite lateral surfaces of the carcass structure 101, in an axially outer position with respect to the carcass structure 101 itself. Each sidewall 108 extends from one of the lateral edges of the tread band 109 up to the respective annular reinforcing structure 103.

The anti-abrasion strip 105, when provided, extends at least up to the respective sidewall 108.

In some specific embodiments, like the one shown and described herein, the rigidity of the sidewall 108 can be improved by providing a stiffening layer 120, generally known as "flipper" or additional strip-like insert, which has the function of increasing the rigidity and integrity of the annular reinforcing structure 103 and of the sidewall 108.

The flipper 120 is wound around a respective bead core 102 and the elastomeric filler 104 so as to at least partially surround the annular reinforcing structure 103. In particular, the flipper 120 wraps around the annular reinforcing structure 103 along the axially inner, axially outer and radially inner zones of the annular reinforcing structure 103.

The flipper 120 is arranged between the turned end edge of the carcass layer 111 and the respective annular reinforcing structure 103. Usually, the flipper 120 is in contact with the carcass layer 111 and the annular reinforcing structure 103.

In some specific embodiments, like the one shown and described herein, the bead structure 103 can also comprise a further stiffening layer 121 that is generally known with the term "chafer", or protective strip, and which has the function of increasing the rigidity and integrity of the annular reinforcing structure 103.

The chafer 121 is associated with a respective turned end edge of the carcass layer 111 in an axially outer position with respect to the respective annular reinforcing structure 103 and extends radially towards the sidewall 108 and the tread band 109.

The flipper 120 and the chafer 121 comprise reinforcing cords 10d (in the attached figures those of the chafer 121 cannot be seen) coated with an elastomeric material or incorporated in a matrix of cross-linked elastomeric material.

The tread band 109 has, in a radially outer position thereof, a rolling surface 109a intended to come into contact with the ground. The rolling surface 109a has circumferential grooves (not shown in FIG. 1) formed on it, which are connected by transversal notches (not shown in FIG. 1) so as to define a plurality of blocks of various shapes and sizes (not shown in FIG. 1) on the rolling surface 109a.

A sub-layer 107 is arranged between the zero degrees belt layer 106c and the tread band 109.

In some specific embodiments, like the one shown and described herein, a strip 110 consisting of elastomeric mate-

## 15

rial, commonly known as "mini-sidewall", can possibly be provided in the connection zone between the sidewalls **108** and the tread band **109**. The mini-sidewall **110** is generally obtained through co-extrusion with the tread band **109** and allows an improvement of the mechanical interaction between the tread band **109** and the sidewalls **108**.

Preferably, an end portion of the sidewall **108** directly covers the lateral edge of the tread band **109**.

In the case of tyres without an air chamber, a layer of elastomeric material **112**, generally known as "liner", can also be provided in a radially inner position with respect to the carcass layer **111** to provide the necessary impermeability to the inflation air of the tyre **100**.

Depending on the type of tyre **100**, the reinforcing cords **10a**, **10b**, **10c**, **10d** can be metallic reinforcing cords **10** made in accordance with the present invention. Such metallic reinforcing cords **10** can also be used in the carcass structure or belt structure of tyres for motorcycle wheels and in the stoneguard layer and/or in the carcass layer or belt layer of tyres for heavy and/or light load vehicle wheels.

An embodiment of a metallic reinforcing cord **10** made in accordance with the present invention is shown in FIG. 2.

With reference to such a figure, the metallic reinforcing cord **10** comprises a plurality of metallic wires **11** (four in the illustrated example) each extending along a longitudinal direction **L** according to a helical geometry defined by a respective helix having a predetermined winding pitch **P**. The metallic reinforcing cord **10** thus extends longitudinally along a helical path with the aforementioned predetermined winding pitch **P**.

With reference to FIGS. 3 and 3a, the metallic reinforcing cord **10** of FIG. 2 is obtained by twisting together, in a conventional twisting machine (not shown in the figures), said plurality of wires **11** and a textile yarn **20** (for example of the type shown in FIG. 3) with a twisting pitch equal to the aforementioned winding pitch **P**, to make an elongated element **15** (for example of the type illustrated in FIG. 3a).

As will be described hereinafter with reference to FIGS. 4 and 5a, 5b, the textile yarn **20** is intended to be removed from the elongated element **15**. After such removal, the metallic wires **11** keep the aforementioned helical geometry and define the metallic reinforcing cord **10**, which will also have a helical geometry.

The metallic wires **11** are preferably all made of the same material, more preferably all made of steel. The metallic wires **11** can be wires made of NT (Normal Tensile) steel or wires made of HT (High Tensile) steel or wires made of ST (Super Tensile) steel or wires made of UT (Ultra Tensile) steel.

The metallic wires **11** have a carbon content lower than or equal to 1, preferably lower than or equal to 0.9%.

Preferably, the carbon content is greater than or equal to 0.7%.

In preferred embodiments, the carbon content is comprised between 0.7% and 1%, preferably between 0.7% and 0.9%.

The metallic wires **11** are typically coated with brass or another corrosion-resistant coating (for example Zn/Mn).

The metallic wires **11** have a diameter preferably greater than, or equal to, 0.04 mm, more preferably greater than, or equal to, 0.08 mm, even more preferably greater than, or equal to, 0.10 mm.

The metallic wires **11** have a diameter preferably lower than, or equal to 0.60 mm, more preferably lower than, or equal to, 0.45 mm.

In preferred embodiments, the metallic wires **11** have a diameter comprised between 0.04 mm and 0.60 mm, pref-

## 16

erably between 0.08 mm and 0.45 mm, even more preferably between 0.10 mm and 0.45 mm.

For example, the metallic wires **11** have a diameter equal to: 0.10 mm, or 0.12 mm, or 0.13 mm, or 0.15 mm, or 0.175 mm, or 0.20 mm, or 0.22 mm, or 0.245 mm, or 0.25 mm, or 0.265 mm, or 0.27 mm, or 0.28 mm, or 0.30 mm, or 0.32 mm, or 0.35 mm, or 0.38 mm, or 0.40 mm, or 0.42 mm, or 0.45 mm.

The number of metallic wires **11** is preferably comprised between 1 and 27.

The textile yarn **20** is preferably made of a water-soluble synthetic polymeric material, even more preferably a polyvinyl alcohol (PVA). Such a textile yarn **20** can be purchased from specialized producers, like for example Kuraray Co., Ltd or Sekisui Specialty Chemicals, or be made by twisting together a plurality of PVA filaments in a conventional twisting machine.

The textile yarn **20** has a diameter preferably greater than, or equal to, 0.15 mm, more preferably greater than, or equal to, 0.30 mm.

The textile yarn **20** has a diameter preferably lower than, or equal to, 2 mm, more preferably lower than, or equal to, 1 mm.

In preferred embodiments, the textile yarn **20** has a diameter comprised between 0.15 mm and 2 mm, preferably between 0.30 mm and 1 mm.

The textile yarn **20** has a linear density preferably greater than, or equal to, 200 dtex, more preferably greater than, or equal to, 700 dtex.

The textile yarn **20** has a linear density preferably lower than, or equal to, 4400 dtex, more preferably lower than, or equal to, 1670 dtex.

In preferred embodiments, the textile yarn **20** has a linear density comprised between 200 dtex and 4400 dtex, preferably between 700 dtex and 1670 dtex.

The metallic reinforcing cord **10** can also comprise a single metallic wire **11**.

The elongated element **15** can comprise more than one textile yarn **20**.

Each metallic wire **11** can be twisted on itself, in the same direction as, or in the opposite direction to, the direction in which it is twisted on the textile yarn **20**.

The winding pitch **P** of the metallic wires **11** is preferably greater than, or equal to, 2 mm, more preferably greater than, or equal to, 4 mm.

The winding pitch **P** of the metallic wires **11** is preferably lower than, or equal to, 50 mm, more preferably lower than, or equal to, 25 mm.

In preferred embodiments, the winding pitch **P** of the metallic wires **11** is comprised between 2 mm and 50 mm, preferably between 4 mm and 25 mm.

The arrangement of the metallic wires **11** about the textile yarn **20** is such that the metallic wires **11** do not completely wrap around the textile yarn **20**. In particular, the metallic wires **11** are arranged around the textile yarn **20** so that, in any cross section of the elongated element **15**, they are at only an angular portion of an ideal circumference that circumscribes the textile yarn **20**. Such an angular portion is defined by an angle that is preferably greater than, or equal to, 15°, more preferably greater than, or equal to, 20°.

Preferably, such an angle is lower than, or equal to, 45°, more preferably lower than, or equal to, 30°.

In preferred embodiments such an angle is comprised between 15° and 45°, more preferably between 20° and 30°.

The metallic reinforcing cord **10** can be obtained from a plurality of elongated elements **15** twisted together.

The metallic wires 11 can be twisted together with the textile yarn 20 with the aforementioned twisting pitch P to form metallic reinforcing cords 10 having a construction of the  $n \times D$  type, where n is the number of metallic wires 11 and D is the diameter of the metallic wires 11.

Examples of metallic reinforcing cords 10 having a construction of the  $n \times D$  type are shown in FIGS. 2, 12, 13, 15, 16, 17 and 20.

The metallic reinforcing cord 10 of FIG. 2 has a  $4 \times D$  construction, whereas the construction of the reinforcing cords of FIGS. 12, 13, 15, 16, 17 and 20 is indicated in the aforementioned figures.

Preferably, in the metallic reinforcing cords 10 having a construction of the  $n \times D$  type, the number of metallic wires 11 is comprised between 2 and 7, more preferably between 2 and 6, even more preferably between 2 and 5. Preferably, all of the metallic wires 11 have the same diameter.

Alternatively, the metallic wires 11 can be twisted together with the aforementioned twisting pitch P to form respective metallic strands 11 that are then twisted together to form the metallic reinforcing cord 10.

Examples of such metallic reinforcing cords 10 are shown in FIGS. 11, 14, 18 and 19. Such metallic reinforcing cords 10 have a construction of the  $m \times n \times D$  type, where m is the number of strands twisted together, n is the number of metallic wires of the respective strand and D is the diameter of the latter. The construction of the reinforcing cords of FIGS. 11, 14, 18 and 19 is indicated in the aforementioned figures.

In the metallic reinforcing cords 10 having a construction of the  $m \times n \times D$  type, the number of strands of metallic wires 11 can be equal to or different from the number of metallic wires of each strand of metallic wires 11.

Preferably, the number of strands of metallic wires 11 is comprised between 3 and 6, more preferably between 2 and 5.

Preferably, the number of metallic wires 11 of each strand of metallic wires 11 is comprised between 2 and 7.

The twisting pitch of the metallic wires of a strand of metallic wires 11 can be equal to or different from that of the metallic wires of another strand of metallic wires 11 and equal to or different from the twisting pitch of the various strands of metallic wires 11.

Preferably, all of the metallic wires of all of the strands of metallic wires 11 have the same diameter, but embodiments are foreseen wherein the metallic wires of a strand of metallic wires 11 have the same diameter, such a diameter being different that of the metallic wires of another strand of metallic wires 11.

Alternatively, the metallic wires 11 can be twisted together so as to take up a geometry like that shown in FIG. 21, or a different geometry like that shown in FIG. 22.

In the embodiment of FIG. 21, the metallic reinforcing cord 10 comprises a substantially straight first metallic wire 11a on which a second metallic wire 11b is wound in a helix with the aforementioned twisting pitch P. The metallic reinforcing cord of FIG. 21 therefore has a  $1+1 \times D$  construction, where D is the diameter of the metallic wires 11a and 11b.

Preferably, in the metallic reinforcing cords having a  $1+1 \times D$  construction, the metallic wires 11a and 11b have the same diameter, but embodiments are foreseen wherein the metallic wires 11a and 11b have different diameters.

Further embodiments are foreseen comprising a plurality of substantially parallel metallic wires 11a and a metallic wire 11b wound in a helix on such metallic wires 11a. Such metallic reinforcing cords 10 have a construction of the

$1+n \times D$  type, where n is the number of metallic wires 11a and D is the diameter of the metallic wires 11a and 11b.

Preferably, in the metallic reinforcing cords 10 having a construction of the  $1+n \times D$  type the number of metallic wires 11a is comprised between 2 and 7, more preferably between 2 and 6.

Preferably, the metallic wires 11a have the same diameter, but embodiments are foreseen wherein the metallic wires 11a and 11b have different diameters.

Alternatively, it is possible to provide metallic reinforcing cords 10 comprising a single substantially straight metallic wire 11a and a plurality of metallic wires 11b wound in a helix on the aforementioned metallic wire 11a. Such metallic reinforcing cords 10 have a construction of the  $n \times 1 \times D$  type, where n is the number of metallic wires 11b and D is the diameter of the metallic wires 11a and 11b.

Preferably, in the metallic reinforcing cords 10 having a construction of the  $n \times 1 \times D$  type the number of metallic wires 11b is comprised between 2 and 7, more preferably between 2 and 6.

Preferably, the metallic wires 11b have the same diameter, but embodiments are foreseen wherein the metallic wires 11a and 11b have different diameters.

In the embodiment of FIG. 22, the metallic reinforcing cord 10 comprises at least two metallic wires 11a, 11b twisted together with the aforementioned twisting pitch to define at least one strand of metallic wires 11. The strand of metallic wires 11 is twisted together with a plurality of metallic wires 12 (in the case shown in FIG. 12, three metallic wires 12) with a twisting pitch P1 that can be equal to or different from the twisting pitch P (in the specific example shown in FIG. 22, P1 is different from P). Such a metallic reinforcing cord 10 has a construction of the  $m+n \times D$  type, where m is the number of strands of metallic wires 11, n is the number of metallic wires and D is the diameter of the metallic wires 11a and 11b.

The metallic reinforcing cord of FIG. 22 has a construction  $1+3 \times D$ .

The number of metallic wires of each strand of metallic wires 11 can be equal to or different from the number of strands of metallic wires 11 and from the number of metallic wires 12.

Preferably, the number of metallic wires of each strand of metallic wires 11 is comprised between 1 and 7.

Preferably, the number of strands of metallic wires 11 is comprised between 1 and 7, more preferably between 1 and 6, even more preferably between 1 and 4.

Preferably, the number of metallic wires 12 is comprised between 2 and 7.

Preferably, the metallic wires 11a, 11b and 12 all have the same diameter, but embodiments are foreseen wherein the metallic wires 12 have a diameter different from that of the metallic wires 11a, 11b.

With reference to FIG. 4, an embodiment of an apparatus for manufacturing the metallic reinforcing cord 10 in accordance with the present invention and an embodiment of a process for manufacturing the metallic reinforcing cord 10 in accordance with the present invention are described. For the sake of simplicity of description, reference will be made to a metallic reinforcing cord 10 consisting of a single metallic wire 11, obtained from a single elongated element 15, the latter being obtained by twisting together said single metallic wire 11 and a single textile yarn 20.

The textile yarn 20 and the metallic wire 11 are taken from respective reels 40 and 30 and fed to a twisting device 60 to be twisted together, so as to form the elongated element 15.

The twisting device 60 is therefore arranged downstream of the reels 40 and 30 with respect to a feeding direction indicated with A in FIG. 4.

The elongated element 15 is fed, along said feeding direction A, to a removal device 70 in which the textile yarn 20 is removed from the elongated element 15, thus obtaining the metallic reinforcing cord 10. The removal device 70 is therefore arranged downstream of the twisting device 60 with respect to the feeding direction A.

In a preferred embodiment of the invention, the removal device 70 comprises a hot water jet feeding device 73 configured to feed a hot water jet against the elongated element 15, in a counter-current while the elongated element 15 moves along the feeding direction A. The hot water jet dissolves the textile yarn 20 while such a jet is crossed by the metallic wire 11, which remains the only constituent element of the metallic reinforcing cord 10.

Preferably, the metallic reinforcing cord 10 thus formed then crosses a drying device 75 to be subsequently wound in a respective collection reel 50, from which it can be taken during the manufacture of the specific structural component of the tyre 100 of interest. The drying device 75 is therefore arranged downstream of the removal device 70 with respect to the feeding direction A.

In the process described above with reference to FIG. 4, the manufacturing of the metallic reinforcing cord 10 is carried out while obtaining the elongated element 15 (and while removing the textile yarn 20). The metallic reinforcing cord 10 is thus made through a continuous process that comprises, in a time sequence free of interruptions or stops, making the elongated element 15 by mutually twisting the metallic wire 11 and the textile yarn 20, moving the elongated element 15 thus made along the feeding direction A, removing the textile yarn 20, possibly drying the metallic reinforcing cord 10 thus formed and winding the metallic reinforcing cord 10 in the collection reel 50.

However, it is possible to manufacture the metallic reinforcing cord 10 in two distinct operative steps, i.e. through a discontinuous process like for example the one shown in FIGS. 5a, 5b. Such a process differs from the one described above with reference to FIG. 4 only in that the elongated element 15, once made, is collected in a service reel 45 (FIG. 5a), from which it can be taken when desired to proceed with the manufacturing of the metallic reinforcing cord 10 as described earlier (FIG. 5b). The service reel 45 is thus intended to be arranged downstream of the twisting device 60 when the elongated element 15 is made and upstream of the removal device 70 when the textile yarn 20 is removed from the elongated element 15 to manufacture the metallic reinforcing cord 10.

The metallic reinforcing cords 10 are intended to be incorporated in a piece of elastomeric material through conventional calendering processes in conventional rubberizing machines to make the various structural components of the tyre 100 described above.

The metallic reinforcing cord 10 can be made with different helical geometries depending on the particular application (type of tyre of interest or structural component thereof of interest). The helical geometry can be changed by intervening on one or more of the following parameters: number of metallic wires 11, 11a, 11b, diameter of the metallic wires 11, 11a, 11b, diameter (or linear density) of the textile yarn 20 (i.e. number of filaments and/or ends of the textile yarn 20), twisting pitch P, number of textile yarns 20, degree of preforming in the twisting device 60 or in the rubberizing machine.

Depending on the predetermined helical geometry the metallic reinforcing cord 10 will have different mechanical behavior that translates, in a load-elongation graph, into a different curve. It is thus possible to manufacture metallic reinforcing cords 10 having different rigidities, breaking loads, elongations at break, penetrations and part load elongations.

FIG. 6 shows a comparative qualitative example of the mechanical behavior of conventional reinforcing cords and of metallic reinforcing cords 10 made in accordance with the present invention.

On the right the load-elongation curves of various metallic reinforcing cords 10 having different helical geometry are shown.

On the left, on the other hand, the load-elongation curves of four conventional reinforcing cords are shown: the curve indicated with 1 is of a HE metallic reinforcing cord comprising three strands of metallic wires twisted together, each strand comprising three wires made of steel having a diameter equal to 0.20 mm (such a curve thus has a construction which can be identified as 3x3x0.20 HE), the curve indicated with 2 is of a HE metallic reinforcing cord comprising three strands of metallic wires twisted together, each strand comprising four steel wires having a diameter equal to 0.20 mm (such a curve thus has a construction which can be identified as 3x4x0.20 HE), the curve indicated with 3 is of a HE metallic reinforcing cord comprising three strands of metallic wires twisted together, each strand comprising seven steel wires having a diameter equal to 0.20 mm (such a curve thus has a construction which can be identified as 3x7x0.20 HE), the curve indicated with 4 is of a hybrid reinforcing cord comprising a textile yarn made of polyester (PES) twisted together with three strands of metallic wires, each strand comprising two steel wires having a diameter equal to 0.15 mm (such a curve thus has a construction which can be identified as PES+3x2x0.15).

FIG. 6 shows that, depending on the predetermined helical geometry (i.e. the construction), the metallic reinforcing cord 10 has a different mechanical behavior, thus being able to achieve rigidities and breaking loads comparable to those of conventional HE metallic reinforcing cords, with part load elongations and/or at break even much greater than those of conventional HE metallic reinforcing cords and of conventional hybrid or mixed textile reinforcing cords.

FIG. 7 shows, as an example, the load-elongation curves of five metallic reinforcing cords 10 made in accordance with the present invention and having different helical geometry:

- the reinforcing cord of the curve indicated with a has a construction (32)+2x0.30 HT;
- the reinforcing cord of the curve indicated with b has a construction (32)+4x0.30 HT;
- the reinforcing cord of the curve indicated with c has a construction (16)+6x0.14 HT;
- the reinforcing cord of the curve indicated with d has a construction (32)+4x0.14 HT;
- the reinforcing cord of the curve indicated with e has a construction (32)+6x0.14 HT.

In the aforementioned constructions the number in brackets indicates the number of ends twisted together to obtain the textile yarn 20 that will then be removed (such a number is thus indicative of the diameter of the textile yarn 20), the number after+indicates the number of metallic wires 11 twisted together with the textile yarn 20, the number after x indicates the diameter of the metallic wires 11 (in mm) and HT indicates the type of steel used.

FIG. 7 shows that it is possible to manufacture metallic reinforcing cords **10** having part load elongations even equal to 12% and elongations at break even equal to 15%. These values are much greater than those obtainable with conventional metallic reinforcing cords; the latter, indeed, typically have values of part load elongation not greater than 3% and values of elongation at break not greater than 5%, in the case of HE metallic reinforcing cords. It should also be noted that, for example, by increasing the number of ends in the textile yarn **20** (and therefore the diameter of the textile yarn **20**) while keeping the other parameters unchanged, the part load elongation and the elongation at break increase, thus keeping the rigidity and the breaking load unchanged (comparison between curves c and e), whereas by decreasing the diameter of the metallic wires **11** while keeping the other parameters unchanged, the part load elongation and the elongation at break increase, thus reducing the rigidity and the breaking load (comparison between curves b and d).

FIG. 8 shows, as an example, the load-elongation curves of a conventional metallic reinforcing cord (curve A) and of two metallic reinforcing cords **10** having different helical geometries (curves B and C). The reinforcing cord of the curve indicated with A has a construction  $3 \times 4 \times 0.175$  HE and a twisting pitch equal to 6.3 mm (it is thus a HE metallic reinforcing cord made by twisting together three strands of metallic wires with a twisting pitch equal to 6.3, each strand comprising four steel wires having a diameter equal to 0.175 mm). The reinforcing cord of the curve indicated with B has a construction  $(36)+3 \times 4 \times 0.175$  HE and a twisting pitch equal to 6.3 mm (it is thus a HE metallic reinforcing cord made by twisting together a cord as described above and a textile yarn having 36 ends twisted together). The reinforcing cord of the curve indicated with C has the same identical construction as the reinforcing cord of the curve indicated with B, except for having a greater twisting pitch (equal to 12.5 mm).

FIG. 8 shows that, while keeping unchanged the twisting pitch, the number of metallic wires, the diameter of the metallic wires and the metallic material, the metallic reinforcing cord **10** made in accordance with the present invention has a part load elongations and an elongation at break much greater than those of a conventional HE metallic reinforcing cord, with no substantial reduction of the rigidity and of the breaking load (comparison between curves A and B). It should also be noted that a change in the helical geometry of the metallic reinforcing cord **10** obtained only by increasing the twisting pitch  $P$  results in a reduction of the part load elongations and elongation at break, also in this case with no substantial reduction of the rigidity and of the breaking load with respect to those of a conventional HE metallic reinforcing cord (comparison between curves B and C).

FIG. 9 shows, as an example, the load-elongation curves of further three metallic reinforcing cords **10** having different helical geometries (curves A, B and C). The reinforcing cord of the curve indicated with A is a HE metallic reinforcing cord made by twisting together three metallic steel wires having a diameter equal to 0.35 mm and a textile yarn having 36 ends twisted together and subjected to conventional preforming systems, in particular of the permanent wave type. Such a cord thus has a construction  $(36)+3 \times 0.35$  HE. The reinforcing cord of the curve indicated with B is a HE metallic reinforcing cord having a construction  $(36)+4 \times 0.35$  HE; it differs from the one discussed above only in that it comprises four metallic wires. The reinforcing cord of the curve indicated with C is a HE metallic reinforcing cord

having a construction  $(36)+5 \times 0.35$  HE; it differs from those discussed above only in that it comprises five metallic wires.

It should be noted that the elongation at break of these reinforcing cords is greater than 6% with a part load elongation varying between 0.2% and 0.7%, whereas the elongation at break of the conventional HE metallic reinforcing cords with identical number and diameter of wires, identical material and identical degree of preforming does not exceed 5%. It should also be noted that when the number of wires increases the breaking load increases as well and, in a less accentuated manner, also the elongation at break increases.

FIG. 10 shows, as an example, the load-elongation curves of a conventional HE metallic reinforcing cord of the  $3 \times 7 \times 0.20$  HE type (curve A) and those of four metallic reinforcing cords **10** having different helical geometries (curves B, C, D, E).

The reinforcing cord of the curve indicated with A is a HE metallic reinforcing cord comprising three strands of metallic wires, each comprising seven metallic wires having a diameter equal to 0.20 mm and a part load elongation increased through preforming. The three strands are twisted together with a twisting pitch equal to 3.15 mm, whereas the seven metallic wires of each strand are twisted together with a twisting pitch equal to 6.3 mm. It thus has a  $3 \times 7 \times 0.20$  HE construction.

The reinforcing cord of the curve indicated with B has the same construction above but it is made from an elongated element obtained by winding the aforementioned strands on a textile yarn having 18 ends twisted together. It thus has a  $(18)+3 \times 7 \times 0.20$  HE construction.

The reinforcing cord of the curve indicated with C has the same construction above but it is made from an elongated element obtained by winding the aforementioned strands on a textile yarn having 36 ends twisted together. It thus has a  $(36)+3 \times 7 \times 0.20$  HE construction.

The reinforcing cord of the curve indicated with D has the same construction above but it is made from an elongated element obtained by winding the aforementioned strands on a textile yarn having 54 ends twisted together. It thus has a  $(54)+3 \times 7 \times 0.20$  HE construction.

The reinforcing cord of the curve indicated with E has the same construction above but it is made from an elongated element obtained by winding the aforementioned strands on a textile yarn having 72 ends twisted together. It thus has a  $(72)+3 \times 7 \times 0.20$  HE construction.

FIG. 10 shows that, while keeping unchanged the twisting pitch, the number of strands and metallic wires in each strand, the diameter of the metallic wires, the metallic material and the degree of preforming, the metallic reinforcing cords **10** made in accordance with the present invention all have part load elongations and elongations at break greater than those of the conventional HE metallic reinforcing cord, with no reduction of rigidity and breaking load. It should also be noted that the part load elongations and elongations at break increase as the number of ends (and therefore the diameter) of the textile yarn used increases.

The graphs discussed above therefore confirm what has already been stated earlier, i.e. that by changing one or more among number of metallic wires **11**, diameter of the metallic wires **11**, diameter (or linear density) of the textile yarn **20** (i.e. number of filaments or ends of the textile yarn **20**), twisting pitch  $P$ , number of textile yarns **20**, degree of preforming in the twisting device **60** or in the rubberizing machine, it is possible to manufacture metallic reinforcing cords **10** having different helical geometries (or constructions), thus being able each time to manufacture a metallic

reinforcing cord **10** having the mechanical behavior deemed most suitable for the tyre of interest or for the structural component of interest.

FIGS. 11-20 show, as examples, various metallic reinforcing cords **10** made in accordance with the present invention and respective conventional metallic reinforcing cords, indicated with STD. All of the illustrated reinforcing cords have a helical geometry, but such helical geometry is different depending on the specific construction of each of the illustrated reinforcing cords.

To the left of each of the illustrated reinforcing cords various cross sections of the reinforcing cord are shown and, to the left of such cross sections the specific construction of the metallic reinforcing cord is given. The twisting pitch in mm is indicated with P and the number of ends of the textile yarn **20** used to manufacture the illustrated metallic reinforcing cords **10** is in brackets.

The reinforcing cords shown in FIG. 11 are HE metallic reinforcing cords each comprising three metallic strands, each comprising four HT steel wires having a diameter equal to 0.175 mm, twisted together with a twisting pitch equal to 6.3 mm.

It should be noted that as the construction changes, the helical geometry of the metallic reinforcing cord **10** and the distribution of the metallic wires in a predetermined piece of elastomeric material change. In particular, unlike the conventional HE metallic reinforcing cord in which the metallic wires (in this case grouped in strands) are collected together and concentrated substantially at the center of the aforementioned piece, in the metallic reinforcing cords **10** made in accordance with the present invention the metallic wires (also grouped in strands) are distributed over a wider area of the aforementioned piece as the diameter of the textile yarn and of the twisting pitch increase.

The reinforcing cords shown in FIG. 12, on the other hand, comprise four HT steel wires having a diameter of 0.30 mm. All of these reinforcing cords have a geometry such that in some or all of their cross sections at least some of the steel wires are in a condition of substantial mutual contact (by this expression meaning both a condition of actual contact of two adjacent steel wires and a condition in which the distance between two adjacent steel wires is much lower than the diameter of the steel wires, in particular equal to or lower than half the diameter of the steel wires, even more in particular lower than one third of the diameter of the steel wires). The two metallic reinforcing cords **10** have a space, defined between the various steel wires and originally occupied by the textile yarn used to manufacture them, which is much greater than that of the conventional metallic reinforcing cord. Such a space increases, while keeping the other parameters unchanged, as the diameter of the textile yarn used increases (and thus as the number of filaments and/or ends of the textile yarn increase). Moving from top to bottom in FIG. 12 the penetration, the elongation at break and the part load elongation increase.

In accordance with the present invention, it is possible to manufacture metallic reinforcing cords **10** having helical geometries such that in all of their cross sections the metallic wires **11** are in a condition of substantial mutual contact, or metallic reinforcing cords **10** having helical geometries such that in first cross sections of the metallic reinforcing cord **10** some or all of the metallic wires **11** are in a condition of substantial mutual contact and in second cross sections of the metallic reinforcing cord **10** some or all of the metallic wires **11** are spaced apart from one another.

The present invention also makes it possible to manufacture metallic reinforcing cords **10** having helical geometries

such that in all of the cross sections of the metallic reinforcing cord **10** all of the metallic wires **11** are spaced apart from one another.

The spacing of the metallic wires **11** can be obtained by suitably deforming (or preforming) the metallic reinforcing cords **10** while they are pulled with a predetermined traction force, which can be constant or variable over time. Such a deformation (or preforming) can be obtained by passing the metallic reinforcing cord **10** over a plurality of cylinders having a reduced diameter (for example comprised between 1 and 5 mm) with a predetermined pull. Such deformation is minimum when cylinders of greater diameter are used and maximum when cylinders of smaller diameter are used.

FIG. 13 shows a conventional metallic reinforcing cord (indicated with STD) and five metallic reinforcing cords **10** made in accordance with the present invention and subjected to suitable deformation so as to space all of the metallic wires from one another. The marking "pref." indicates the degree of deformation (minimum or maximum) to which the metallic reinforcing cord **10** has been subjected to have all of the metallic wires spaced apart from each other.

All of the reinforcing cords shown in FIG. 13 comprise five UT steel wires having a diameter equal to 0.22 mm.

It should be noted that, while keeping the other parameters unchanged, as the twisting pitch P increases the helical geometry of the metallic reinforcing cord **10** and the distribution of the metallic wires in a predetermined piece of elastomeric material change. In particular, unlike the conventional metallic reinforcing cord in which the metallic wires are collected together and concentrated substantially at the center of the aforementioned piece, in the metallic reinforcing cords **10** the metallic wires are distributed over the entire volume of the aforementioned piece.

It should also be noted that, while keeping the other parameters unchanged, the greater the deformation, the greater the distribution of the metallic wires over the entire volume of the piece of elastomeric material (comparison between the last two reinforcing cords at the bottom of FIG. 11). The degree of deformation imparted on the metallic reinforcing cord **10** can thus also be considered as a useful parameter on which to intervene to provide the metallic reinforcing cord **10** with the helical geometry (and therefore the mechanical behavior) deemed ideal for the particular application required.

The distribution of the metallic wires inside the aforementioned structural component can be changed by changing, over time, the amount of the traction force with which the metallic reinforcing cord **10** is pulled during the aforementioned deformation or during the process of incorporation of the metallic reinforcing cord **10** in the piece of elastomeric material to make the structural component of interest of the tyre.

In accordance with the present invention, since it is possible to have very large twisting pitches (for example equal to 35 mm) with no risk of unravelling, it is possible to manufacture very flat metallic reinforcing cords **10**. This makes it possible to double, or more generally multiply, the number of metallic reinforcing cords provided in a specific portion of piece of structural component with respect to the case where conventional metallic reinforcing cords are used.

FIG. 14 shows the HE metallic reinforcing cords discussed with reference to FIG. 10.

FIG. 15 shows four metallic reinforcing cords **10** made in accordance with the present invention. In order to manufacture each of such metallic reinforcing cords **10** two textile yarns were used, each comprising 16 ends twisted together (first and third cord in FIG. 15 moving from top to bottom)

or 36 ends twisted together (second and fourth cord in FIG. 15 moving from top to bottom). The two textile yarns were twisted together with four UT steel wires having a diameter equal to 0.30 mm. It should be noted that as the number of ends of the textile yarn and the twisting pitch increase the metallic wires tend to be arranged almost parallel. In this case, the part load elongation is low but the machine output increases.

Similar considerations on the correlation between twisting pitch and machine output and/or between number of ends of the textile yarn and machine output can be made with reference to the metallic reinforcing cords 10 shown in FIGS. 16-20. The first reinforcing cord shown in each of the aforementioned figures is a conventional metallic reinforcing cord, indicated with STD. The construction of each of the reinforcing cords shown in FIGS. 16-20 is clear in light of the indications given in the aforementioned figures alongside the aforementioned reinforcing cords and of the examples discussed above.

The Applicant has made further examples of metallic reinforcing cords 10 and has compared the mechanical behavior of these reinforcing cords with that of hybrid and conventional metallic reinforcing cords. The result of the comparison is indicated in table 1 below.

TABLE 1

|                         | Breaking load (N) | Elongation at break (%) | Part Load Elongation (%) |
|-------------------------|-------------------|-------------------------|--------------------------|
| (36 + 36) + 4 x 0.30 UT | 979               | 4.8                     | 2.68                     |
| (16 + 16) + 4 x 0.30 UT | 981               | 3.69                    | 1.51                     |
| (16) + 6 x 0.30 HT      | 1062              | 5.48                    | 1.40                     |
| (32) + 6 x 0.30 HT      | 1113              | 9.85                    | 2.37                     |
| PES + 5 x 0.28          | 907               | 3.62                    | 0.54                     |
| PES + 5 x 0.25          | 729               | 3.99                    | 0.74                     |

In table 1, the first four cords are metallic reinforcing cords 10 in accordance with the present invention whereas the last two cords are conventional reinforcing cords. These last two conventional reinforcing cords are hybrid reinforcing cords comprising a textile yarn made of polyester (PES) twisted together with five metallic wires having a diameter equal to 0.28 mm (the penultimate cord in table 1) and 0.25 mm (the last cord in table 1).

In the first two metallic reinforcing cords 10 of table 1 the Applicant has used two textile yarns, each respectively comprising 36 ends (in the first reinforcing cord) and 16 ends (in the second reinforcing cord). Such textile yarns were twisted together with four UT steel wires having a diameter equal to 0.30 mm. In the third and fourth metallic reinforcing cord 10 of table 1 the Applicant has used a single textile yarn comprising 16 ends (in the third reinforcing cord) and 32 ends (in the fourth reinforcing cord). Such a textile yarn was twisted together with six UT steel wires having a diameter equal to 0.30 mm.

It should be noted that some of the metallic reinforcing cords 10 of table 1 have a (and even much greater) part load elongation and elongation at break greater than those of conventional hybrid or metallic reinforcing cords, with substantially identical rigidity and breaking load.

The Applicant made further examples of metallic reinforcing cords 10 and has compared the mechanical behavior of these reinforcing cords with those of a conventional HE metallic reinforcing cord of analogous construction. All of these metallic reinforcing cords comprise three strands twisted together, each strand comprising seven metallic

wires having a diameter equal to 0.20 mm (such metallic reinforcing cord thus have a 3x7x0.20 HE construction). The strands are twisted together with a first twisting pitch, whereas the metallic wires in each strand are twisted together with a second twisting pitch. The result of the comparison is indicated in table 2 below.

TABLE 2

|                                | Breaking load (N) | Elongation at break (%) | Part Load Elongation (%) |
|--------------------------------|-------------------|-------------------------|--------------------------|
| 3 x 7 x 0.20 HE                | 1833              | 4.19                    | 1.87                     |
| 1 + 1 x (36) + 3 x 7 x 0.20 HE | 1617              | 14.58                   | 4.16                     |
| 3 x (36) + 3 x 7 x 0.20 HE     | 1827              | 5.04                    | 2.40                     |
| 1 + 2 x (36) + 3 x 7 x 0.20 HE | 1817              | 12.40                   | 6.78                     |
| 1 + 3 x (36) + 3 x 7 x 0.20 HE | 1844              | 12.97                   | 6.89                     |

In table 2, the first cord is a conventional metallic reinforcing cord, whereas the other four cords are metallic reinforcing cords 10 in accordance with the present invention: they differ from each other by the type of textile yarn used to manufacture them.

In the conventional metallic reinforcing cord, the first twisting pitch is equal to 3.8 mm, whereas the second twisting pitch is equal to 6.3 mm.

In the metallic reinforcing cord 10 having the construction 1+1x(36)+3x7x0.20 HE a central textile yarn comprising 36 ends and a crown textile yarn comprising 36 ends are used. These two textile yarns are twisted together with the aforementioned strands of metallic wires. The first twisting pitch is equal to 3.15 mm, whereas the second twisting pitch is equal to 6.3 mm.

In the metallic reinforcing cord 10 having the construction 3x(36)+3x7x0.20 HE three textile yarns are used, each comprising 36 ends. Such textile yarns are twisted together with the aforementioned strands of metallic wires. The first twisting pitch is equal to 4.2 mm, whereas the second twisting pitch is equal to 12.5 mm.

In the metallic reinforcing cord 10 having the construction 1+2x(36)+3x7x0.20 HE a central textile yarn comprising 36 ends and two crown textile yarns each comprising 36 ends are used. These three textile yarns are twisted together with the aforementioned strands of metallic wires. The first twisting pitch is equal to 4.2 mm, whereas the second twisting pitch is equal to 12.5 mm.

In the metallic reinforcing cord 10 having the construction 1+3x(36)+3x7x0.20 HE a central textile yarn comprising 36 ends and three crown textile yarns each comprising 36 ends are used. These four textile yarns are twisted together with the aforementioned strands of metallic wires. The first twisting pitch is equal to 4.2 mm, whereas the second twisting pitch is equal to 12.5 mm.

It should be noted that some of the metallic reinforcing cords 10 have an elongation at break greater (and even much greater, see the values 12.4% and 14.58%) than that of the conventional metallic reinforcing cord, with a substantially identical rigidity and breaking load.

The Applicant has made further examples of metallic reinforcing cords 10 deemed suitable for being used in the carcass and has evaluated their breaking load and the respective elongation at break. Such reinforcing cords and the result of the aforementioned evaluation is indicated in table 3 below.

Each of the two cords indicated in table 3 comprises twelve metallic wires made of UT steel having a diameter equal to 0.22 mm and twisted together with a predetermined

twisting pitch. These cords are obtained by twisting together the aforementioned metallic wires and a textile yarn (which is then removed) comprising 16 ends twisted together, with a twisting pitch equal to 12.5 mm. The two cords differ from each other only in that in the second the metallic wires have been subjected to a preforming before being twisted together with the textile yarn.

TABLE 3

|                     | Breaking load (N) | Elongation at break (%) | Part Load Elongation (%) |
|---------------------|-------------------|-------------------------|--------------------------|
| (16) + 12 x 0.22 UT | 1611              | 3.57                    | 1.06                     |
| (16) + 12 x 0.22 UT | 1604              | 4.64                    | 1.76                     |

The Applicant has observed that typically the metallic reinforcing cords used in the carcass structure of the tyres do not allow a suitable penetration of the surrounding elastomeric material due to their particularly closed geometry. In such reinforcing cords typically the metallic wires would be in mutual contact and thus subject to the undesired phenomenon of fretting, at the expense of the structural integrity of the tyre.

The metallic reinforcing cords **10** made in accordance with the present invention (like for example the two cords indicated in table 3) on the other hand, thanks to the free space obtained through the removal of the textile yarn and to the possibility of spacing apart the various metallic wires, allow adequate penetration of the elastomeric material inside the cord and prevent the mutual contact of the various metallic wires, at the same time reaching values of breaking load, elongation at break and part load elongations which are more than acceptable for the specific application. It is thus possible to achieve the desired structural integrity of the tyre with a smaller number of metallic wires in the carcass structure or, the number of metallic wires being equal, with metallic wires having a smaller diameter, with consequent advantages in terms of weight and cost of the tyre.

All of the example discussed above and shown in the attached figures demonstrate just how large is the possibility of manufacturing, through the process and/or the apparatus of the present invention, metallic reinforcing cords **10** having different mechanical behaviors, making it possible to identify each time the ideal one for the specific application. In particular, the reinforcing cords **10** can be used in the crossed belt structure and/or in the chafer and/or in the flipper and/or in the zero degrees belt layer of tyres for automobiles, in the zero degrees belt layer and/or in the chafer and/or in the flipper of tyres for motorcycles and in the carcass structure and/or in the crossed belt structure and/or in the chafer and/or in the flipper and/or in the zero degrees belt layers and/or in the stoneguard layer of tyres for heavy and/or light load vehicles.

Among the particularly advantageous aspects thereof, the present invention makes it possible, in preferred embodiments thereof, to manufacture metallic reinforcing cords **10** for tyres for automobiles, motorcycles and heavy and/or light load vehicles that comprise at least one metallic wire **11** that extends along a helical path, preferably at least two metallic wires **11** twisted together with a predetermined twisting pitch, and have a part load elongation preferably greater than 1%, more preferably greater than 2%, more preferably greater than 3%, even more preferably greater than 3.5%, even more preferably greater than 4%, and/or an elongation at break preferably greater than 5%, more preferably lower than 20%, even more preferably up to 15%,

and/or wherein said at least one metallic wire **11** has a winding pitch (or, in the case of a plurality of metallic wires, they are twisted together with a twisting pitch) that is preferably greater than 2 mm, more preferably greater than 3 mm, even more preferably greater than 4 mm, even more preferably greater than 5 mm, allowing values of part load elongation and of elongation at break to be reached such as to be able to use such reinforcing cords also in types of tyres and/or in structural components of tyres in which it has not been possible to use conventional metallic reinforcing cords yet.

This is what also emerged from a series of comparative laboratory tests carried out by the Applicant. Such tests demonstrated that the elongation at break and the part load elongation of metallic reinforcing cords **10** made in accordance with the present invention can reach values even much greater than those of the corresponding conventional metallic reinforcing cords.

Hereinafter, all of the ranges of values are obtained 20 considering all of the following combinations of diameter of the metallic wires **11** and number of metallic wires **11**: minimum diameter and minimum number of metallic wires **11**, maximum diameter and minimum number of metallic wires **11**, minimum diameter and maximum number of metallic wires **11**, maximum diameter and maximum number of metallic wires **11**.

The Applicant simulated the mechanical behavior of metallic reinforcing cords **10** having a  $n \times D$  construction, comprising a plurality of metallic wires **11** twisted together, preferably with a single twisting pitch, where  $n$  is the 30 number of such metallic wires **11**, preferably comprised between 2 and 6, for example equal to 2 or 3 or 4, and  $D$  is the diameter of the metallic wires **11**, selected among any of the diameter values cited above and preferably equal for all 35 of the metallic wires **11** of the metallic reinforcing cord **10**. The Applicant compared the mechanical behavior of such metallic reinforcing cords **10** with that of corresponding conventional metallic reinforcing cords having the same construction and measured, for the conventional metallic 40 reinforcing cords, values of elongation at break comprised in the range 1.5%-2.0% and values of part load elongation comprised in the range 0.2%-0.8%, whereas for the metallic reinforcing cords **10** made in accordance with the present invention the values of elongation at break were comprised 45 in the range 1.5%-15% and those of part load elongation were comprised in the range 0.2%-10%. According to the Applicant, metallic reinforcing cords **10** having the aforementioned construction have a particularly preferred application in the crossed belt structure and/or in the chafer and/or flipper and/or in the zero degrees belt layer of tyres for automobiles, in the zero degrees belt layer and/or in the chafer and/or flipper of tyres for motorcycles, in the crossed 50 belt structure and/or in the chafer and/or flipper and/or in the zero degrees belt layers and/or in the stoneguard layer of tyres for heavy and/or light load vehicles and, with a number of metallic wires **11** greater than 6, preferably greater than or equal to 9, also in the carcass structure of tyres for heavy and/or light load vehicles.

The Applicant also simulated the mechanical behavior of 55 metallic reinforcing cords **10** having a  $n+1 \times D$  or  $1+n \times D$  construction, comprising a strand of metallic wires **11** twisted together with a first twisting pitch, the strand being twisted together with a single metallic wire **11** with a second twisting pitch that can be equal to or different from the first 60 twisting pitch, preferably equal, where  $n$  is the number of metallic wires **11** of the strand, which preferably is comprised between 1 and 6, for example equal to 1 or 2, and  $D$

is the diameter of the metallic wires 11, selected among any of the diameter values cited above, preferably equal for all of the metallic wires 11 of the strand and not necessarily equal to that of the single metallic wire 11. The Applicant compared the mechanical behavior of such metallic reinforcing cords 10 with that of corresponding conventional metallic reinforcing cords having the same construction and measured, for the conventional metallic reinforcing cords, values of elongation at break comprised in the range 1.3%-1.8% and values of part load elongation comprised in the range 0.2%-0.7%, whereas for the metallic reinforcing cords 10 made in accordance with the present invention the values of elongation at break were comprised in the range 1.3%-10% and the values of part load elongation were comprised in the range 0.2%-8.0%. According to the Applicant, metallic reinforcing cords 10 having the aforementioned construction have a particularly preferred application in the crossed belt structure and/or in the chafer and/or flipper and/or in the zero degrees belt layer of tyres for automobiles, in the zero degrees belt layer and/or in the chafer and/or flipper of tyres for motorcycles, in the crossed belt structure and/or in the chafer and/or flipper and/or in the zero degrees belt layers and/or in the stoneguard layer of tyres for heavy and/or light load vehicles and, with a number of metallic wires 11 greater than 6, preferably greater than or equal to 9, also in the carcass structure of tyres for heavy and/or light load vehicles.

The Applicant also simulated the mechanical behavior of metallic reinforcing cords 10 having a  $m+n \times D$  construction, comprising a strand of metallic wires 11 twisted together with a first twisting pitch, the strand being twisted together with a plurality of other metallic wires 11 with a second twisting pitch that can be equal to or different from the first twisting pitch (preferably equal), where  $m$  is the number of metallic wires 11 of the strand, which preferably is comprised between 1 and 6, for example equal to 2 or 3 or 4, and  $n$  is the number of the other metallic wires 11, which preferably is comprised between 1 and 6, for example equal to 2 or 3, and where  $D$  is the diameter of the metallic wires 11, selected among any of the diameter values cited above, preferably equal for all of the metallic wires 11 of the strand and not necessarily equal to that of the other metallic wires 11. The Applicant compared the mechanical behavior of such metallic reinforcing cords 10 with that of corresponding conventional metallic reinforcing cords having the same construction and measured, for the conventional metallic reinforcing cords, values of elongation at break comprised in the range 1.5%-2.0% and values of part load elongation comprised in the range 0.2%-0.8%, whereas for the metallic reinforcing cords 10 made in accordance with the present invention the values of elongation at break were comprised in the range 1.5%-15% and those of part load elongation were comprised in the range 0.2%-10%. According to the Applicant, metallic reinforcing cords 10 having the aforementioned construction have a particularly preferred application in the crossed belt structure and/or in the chafer and/or flipper and/or in the zero degrees belt layer of tyres for automobiles, in the zero degrees belt layer and/or in the chafer and/or flipper of tyres for motorcycles, in the crossed belt structure and/or in the chafer and/or flipper and/or in the zero degrees belt layer and/or in the stoneguard layer of tyres for heavy and/or light load vehicles and, with a number of metallic wires 11 greater than 6, preferably greater than or equal to 9, also in the carcass structure of tyres for heavy and/or light load vehicles.

The Applicant also simulated the mechanical behavior of metallic reinforcing cords 10, preferably of the HE type,

having a  $m \times n \times D$  construction, comprising a plurality of strands of metallic wires 11 twisted together with a first twisting pitch, each strand comprising a plurality of metallic wires twisted together with a second twisting pitch that can be equal to or different from the first twisting pitch (preferably equal), where  $m$  is the number of strands, which preferably is comprised between 2 and 5, for example equal to 2 or 3 or 5, and  $n$  is the number of metallic wires 11 of each strand, which preferably is comprised between 2 and 7 and may or may not be equal to  $m$ , for example equal to 2 or 3 or 6 or 7, where  $D$  is the diameter of the metallic wires 11 preferably equal for all of the metallic wires 11 of all of the strands. The Applicant compared the mechanical behavior of such metallic reinforcing cords 10 with that of corresponding conventional metallic reinforcing cords having the same construction and measured, for the conventional metallic reinforcing cords, values of elongation at break comprised in the range 2.0%-4.5% and values of part load elongation comprised in the range 1.0%-2.5%, whereas for the metallic reinforcing cords 10 made in accordance with the present invention the values of elongation at break were comprised in the range 2.0%-15% and those of part load elongation were comprised in the range 1.0%-7.0%. According to the Applicant, metallic reinforcing cords 10 having the aforementioned construction have a particularly preferred application in the crossed belt structure and/or in the chafer and/or flipper and/or in the zero degrees belt layer of tyres for automobiles, in the zero degrees belt layer and/or in the chafer and/or flipper of tyres for motorcycles, in the crossed belt structure and/or in the chafer and/or flipper and/or in the zero degrees belt layers and/or in the stoneguard layer of tyres for heavy and/or light load vehicles and, with a number of metallic wires 11 greater than 6, preferably greater than or equal to 9, also in the carcass structure of tyres for heavy and/or light load vehicles.

The Applicant also simulated the mechanical behavior of metallic reinforcing cords 10, preferably of the HE type or preformed, having a  $n \times D$  construction, comprising a plurality of metallic wires 11 twisted together, preferably with a single twisting pitch, where  $n$  is the number of such metallic wires 11, preferably comprised between 2 and 6, for example equal to 3, 4 or 5, and  $D$  is the diameter of the metallic wires 11, selected among any of the diameter values cited above and preferably equal for all of the metallic wires 11 of the metallic reinforcing cord 10. The Applicant compared the mechanical behavior of such metallic reinforcing cords 10 with that of corresponding conventional metallic reinforcing cords having the same construction. Depending on the diameter of the metallic wires selected each time, the Applicant measured, for the conventional metallic reinforcing cords, values of elongation at break comprised in the range 3.0%-6.0% and values of part load elongation comprised in the range 0.2%-0.5%, whereas for the metallic reinforcing cords 10 made in accordance with the present invention the values of elongation at break were comprised in the range 3.0%-8.0% and those of part load elongation were comprised in the range 0.2%-1.0%. According to the Applicant, metallic reinforcing cords 10 having the aforementioned construction have a particularly preferred application in the zero degrees belt layer and/or in the chafer and/or flipper of tyres for motorcycles and/or in the crossed belt structure and/or in the zero degrees belt layers and/or in the stoneguard layer and/or in the chafer and/or flipper of tyres for heavy and/or light load vehicles and, with a number of metallic wires 11 greater than 6, preferably greater than or equal to 9, also in the carcass structure of tyres for heavy and/or light load vehicles.

With particular reference to the applications in tyres for heavy and/or light load vehicles, the Applicant also carried out the following comparative laboratory tests.

The Applicant simulated the mechanical behavior of metallic reinforcing cords **10** having constructions of the  $1+n \times D$  type similar to the  $1+n \times D$  constructions cited above, where  $n$  is lower than or equal to 6. The Applicant compared the mechanical behavior of such metallic reinforcing cords **10** with that of corresponding conventional metallic reinforcing cords having the same construction and measured, for the conventional metallic reinforcing cords, values of elongation at break comprised in the range 3.0%-6.0% and values of part load elongation comprised in the range 0.2%-0.5%, whereas for the metallic reinforcing cords **10** made in accordance with the present invention the values of elongation at break were comprised in the range 3.0%-8.0% and the values of part load elongation were comprised in the range 0.2%-1.0%. According to the Applicant, metallic reinforcing cords **10** having the aforementioned construction have a particularly preferred application in the crossed belt structure and/or in the stoneguard layer and/or in the zero degrees belt layers and/or in the chafer and/or flipper of tyres for heavy and/or light load vehicles.

The Applicant also simulated the mechanical behavior of metallic reinforcing cords **10** having constructions of the  $1+n \times D$  type similar to the constructions  $1+n \times D$  cited above, but where  $n$  is greater than 6, preferably greater than or equal to 9, for example equal to 18. The Applicant compared the mechanical behavior of such metallic reinforcing cords **10** with that of corresponding conventional metallic reinforcing cords having the same construction and measured, for the conventional metallic reinforcing cords, values of elongation at break comprised in the range 1.0%-2.0% and values of part load elongation comprised in the range 0%-0.1%, whereas for the metallic reinforcing cords **10** made in accordance with the present invention the values of elongation at break were comprised in the range 1.0%-2.5% and the values of part load elongation were comprised in the range 0%-0.5%. According to the Applicant, metallic reinforcing cords **10** having the aforementioned construction can have a preferred application also in the carcass structure of tyres for heavy and/or light load vehicles.

The Applicant also simulated the mechanical behavior of metallic reinforcing cords **10** having constructions of the  $m+n \times D$  type similar to the  $m+n \times D$  constructions cited above, where  $m$  is equal to 1 or 2 and the twisting pitch of the metallic wires **11** of the strand is different from that of the other metallic wires **11**. The Applicant compared the mechanical behavior of such metallic reinforcing cords **10** with that of corresponding conventional metallic reinforcing cords having the same construction and measured, for the conventional metallic reinforcing cords, values of elongation at break comprised in the range 3.0%-6.0% and values of part load elongation comprised in the range 0.2%-0.5%, whereas for the metallic reinforcing cords **10** made in accordance with the present invention the values of elongation at break were comprised in the range 3.0%-8.0% and the values of part load elongation were comprised in the range 0.2%-1.0%. According to the Applicant, metallic reinforcing cords **10** having the aforementioned construction have a particularly preferred application in the crossed belt structure and/or in the chafer and/or flipper and/or in the zero degrees belt layers and/or in the stoneguard layer of tyres for heavy and/or light load vehicles and, in the case in which  $m$ ,  $n$  or  $m+n$  is greater than 6, preferably greater than or equal to 9, also in the carcass structure of such tyres.

The Applicant also simulated the mechanical behavior of metallic reinforcing cords **10** having constructions of the  $m+n \times D$  type similar to the  $m+n \times D$  constructions cited above, but where  $m$  is equal to 3 and  $n$  is lower than 6. The Applicant compared the mechanical behavior of such metallic reinforcing cords **10** with that of corresponding conventional metallic reinforcing cords having the same construction and measured, for the conventional metallic reinforcing cords, values of elongation at break comprised in the range 1.5%-2.5% and values of part load elongation comprised in the range 0.1%-0.2%, whereas for the metallic reinforcing cords **10** made in accordance with the present invention the values of elongation at break were comprised in the range 1.5%-4.0% and the values of part load elongation were comprised in the range 0.1%-0.8%. According to the Applicant, metallic reinforcing cords **10** having the aforementioned construction have a particularly preferred application in the crossed belt structure and/or in the chafer and/or flipper and/or in the stoneguard layer and/or in the zero degrees belt layers of tyres for heavy and/or light load vehicles.

The Applicant also simulated the mechanical behavior of metallic reinforcing cords **10** having constructions of the  $m+n \times D$  type similar to the  $m+n \times D$  constructions cited above, but where  $m$  is equal to 3 and  $n$  is greater than 6, for example equal to 8 or 9. The Applicant compared the mechanical behavior of such metallic reinforcing cords **10** with that of corresponding conventional metallic reinforcing cords having the same construction and measured, for the conventional metallic reinforcing cords, values of elongation at break comprised in the range 1.5%-2.5% and values of part load elongation comprised in the range 0.1%-0.2%, whereas for the metallic reinforcing cords **10** made in accordance with the present invention the values of elongation at break were comprised in the range 1.5%-4.0% and the values of part load elongation were comprised in the range 0.1%-0.8%. According to the Applicant, metallic reinforcing cords **10** having the aforementioned construction have a particularly preferred application in the carcass structure, in the crossed belt structure and/or in the chafer and/or flipper and/or in the stoneguard layer and/or in the zero degrees belt layers of tyres for heavy and/or light load vehicles.

The Applicant also simulated the mechanical behavior of metallic reinforcing cords **10** having constructions of the  $n \times D$  type similar to the  $n \times D$  constructions cited above, but where  $n$  is greater than 6, for example equal to 11 or 12. The Applicant compared the mechanical behavior of such metallic reinforcing cords **10** with that of corresponding conventional metallic reinforcing cords having the same construction and measured, for the conventional metallic reinforcing cords, values of elongation at break comprised in the range 1.5%-2.5% and values of part load elongation comprised in the range 0.1%-0.2%, whereas for the metallic reinforcing cords **10** made in accordance with the present invention the values of elongation at break were comprised in the range 1.5%-4.0% and the values of part load elongation were comprised in the range 0.1%-0.8%. According to the Applicant, metallic reinforcing cords **10** having the aforementioned construction have a particularly preferred application in the carcass structure and/or in the crossed belt structure and/or in the chafer and/or flipper and/or in the stoneguard layer and/or in the zero degrees belt layers of tyres for heavy and/or light load vehicles.

The Applicant also simulated the mechanical behavior of metallic reinforcing cords **10** having constructions of the  $1+m+n \times D$  or  $2+m+n \times D$  type, comprising one metallic wire **11**, or two metallic wires **11**, or three metallic wires **11**

twisted together with a first twisting pitch, such metallic wire(s) **11** being twisted together with a first strand of metallic wires **11** with a first twisting pitch of the strand that can be equal to or different from said first twisting pitch and with a second strand of metallic wires **11** with a second predetermined twisting pitch of the strand that can be equal to or different from the first twisting pitch and that is preferably different from the first twisting pitch of the strand, where  $m$  is the number of metallic wires **11** of the first strand and  $n$  is the number of metallic wires of the second strand, and  $D$  is the diameter of the metallic wires **11**, selected among any of the diameter values cited above, preferably equal for all of the metallic wires **11** of the metallic reinforcing cord **10**. The Applicant compared the mechanical behavior of such metallic reinforcing cords **10** with that of corresponding conventional metallic reinforcing cords having the same construction and measured, for the conventional metallic reinforcing cords, values of elongation at break comprised in the range 1.0%-2.0% and values of part load elongation comprised in the range 0%-0.1%, whereas for the metallic reinforcing cords **10** made in accordance with the present invention the values of elongation at break were comprised in the range 1.0%-2.5% and the values of part load elongation were comprised in the range 0%-0.5%. According to the Applicant, metallic reinforcing cords **10** having the aforementioned construction have a particularly preferred application in the carcass structure and/or in the crossed belt structure and/or in the chafer and/or flipper and/or in the stoneguard layer and/or in the zero degrees belt layers of tyres for heavy and/or light load vehicles.

The Applicant also simulated the mechanical behavior of metallic reinforcing cords **10** having constructions of the  $n \times D$  type similar to the  $n \times D$  constructions cited above, but where  $n$  is greater than 18, for example equal to 27. The Applicant compared the mechanical behavior of such metallic reinforcing cords **10** with that of corresponding conventional metallic reinforcing cords having the same construction and measured, for the conventional metallic reinforcing cords, values of elongation at break comprised in the range 1.0%-2.0% and values of part load elongation comprised in the range 0%-0.1%, whereas for the metallic reinforcing cords **10** made in accordance with the present invention the values of elongation at break were comprised in the range 1.0%-2.5% and the values of part load elongation were comprised in the range 0%-0.5%. According to the Applicant, metallic reinforcing cords **10** having the aforementioned construction have a particularly preferred application in the carcass structure of tyres for heavy and/or light load vehicles.

The Applicant believes that in tyres for automobiles it is particularly preferred to use metallic reinforcing cords **10** having a  $n \times D$  or  $m \times n \times D$  construction. The main advantages offered by the use of such reinforcing cords are the high capability of penetration of the elastomeric material between the various metallic wires **11**, the high elongation at break, with consequent high rigidity, and the high part load elongation. Such advantages produce benefits in terms of performance, also at high speeds. For applications in the zero degrees belt layers it is also deemed particularly preferred to use metallic reinforcing cords **10** having a  $m \times n \times D$  construction.

In the previous paragraph and in the subsequent ones, the terms "high" should not necessarily be interpreted in absolute terms but rather also in relative terms with respect to the corresponding features of the conventional metallic reinforcing cords having the same construction. Therefore, with reference for example to the part load elongations, it is

considered high simply when it is higher than that of the corresponding conventional metallic reinforcing cords.

The Applicant also believes that in tyres for motorcycles it is particularly preferred to use metallic reinforcing cords **10** having a  $n \times D$  or  $m \times n$  construction. In this case, the main advantages offered by the use of such reinforcing cords are the high capability of penetration of the elastomeric material between the various metallic wires **11** and the high part load elongation, with consequent high rigidity. Such advantages produce benefits in terms of weight and performance. A further advantage offered by such reinforcing cords, the elongation at break being equal to that of the conventional HE or preformed metallic reinforcing cords, is the increase of the machine output, with consequent economic and production benefits.

The Applicant also believes that in the carcass structure of tyres for heavy and/or light load vehicles it is particularly preferred to use metallic reinforcing cords **10** having a  $1+n \times D$  or  $m+n+p$  (i.e., wherein a strand of  $m$  metallic wires **20** is twisted together with  $n$  metallic wires with a first twisting pitch to form an assembly that is then twisted together with  $p$  metallic wires with a second twisting pitch different from the first twisting pitch) or  $n \times D$  construction. In this case, the main advantage offered by the use of such reinforcing cords **25** is the high capability of penetration of the elastomeric material between the various metallic wires **11**, with consequent benefits in terms of fatigue resistance and integrity of the tyre, and thus of mileage.

As to the tyres for heavy and/or light load vehicles, the **30** Applicant believes that it is particularly preferred to use, in their crossed belt structures, metallic reinforcing cords **10** having a  $1+n \times D$  or  $2+n \times D$  or  $3+n \times D$  construction. Also in this case, the main advantage offered by the use of such reinforcing cords is the high capability of penetration of the **35** elastomeric material between the various metallic wires **11**, with consequent benefits in terms of resistance to detachment phenomena of the elastomeric material from the metallic wires of the crossed belt structure during the reconstruction of the tyre.

**40** The Applicant believes that it is particularly preferred to use in the zero degrees belt layers of the tyres for heavy and/or light load vehicles, metallic reinforcing cords **10** having a  $n \times D$  or  $m \times n \times D$  construction (where  $n$  can also be equal to  $m$ ). In this case, the main advantages offered by the **45** use of such reinforcing cords are the high capability of penetration of the elastomeric material between the various metallic wires **11**, the high elongation at break, with consequent high rigidity and the high part load elongation. Such advantages product benefits in terms of performance. A further advantage offered by such reinforcing cords, the elongation at break being equal to that of conventional preformed or HE metallic reinforcing cords, is the increase of the machine output, with consequent economic and production benefits.

**55** The Applicant believes that it is particularly preferred to use in the stoneguard layers of the tyres for heavy and/or light load vehicles, metallic reinforcing cords **10** having a  $n \times$  and  $m \times n \times D$  construction (where  $n$  can also be equal to  $m$ ). In this case, the main advantage offered by the use of such **60** reinforcing cords is the high capability of penetration of the elastomeric material between the various metallic wires **11**, with consequent benefits in terms of performance, comfort and impact resistance. A further advantage offered by such reinforcing cords, the elongation at break being equal to that of conventional preformed or HE metallic reinforcing cords, is the increase of the machine output, with consequent economic and production benefits.

## 35

The Applicant believes that it is particularly preferred to use in the chafer and/or flipper of the tyres for heavy and/or light load vehicles, metallic reinforcing cords **10** having a  $m \times n \times D$  (where  $n$  can also be equal to  $m$ ) or  $1+n \times D$  or  $2+n \times D$  or  $3+n \times D$  construction. In this case, the main advantage offered by the use of such reinforcing cords is the high part load elongation, with consequent benefits in terms of flexibility of such structures, and therefore of resistance to fatigue stresses, which implies an improvement in performance. A further advantage offered by such reinforcing cords, the elongation at break being equal to that of conventional preformed or HE metallic reinforcing cords, is the increase of the machine output, with consequent economic and production advantages.

The present invention has been described with reference to some preferred embodiments. Different changes can be made to the embodiments described above, while remaining within the scope of protection of the invention as defined by the following claims.

The invention claimed is:

**1.** A process for manufacturing a structural component of a tyre for vehicle wheels, comprising:

providing at least one elongated element comprising at least one metallic wire twisted together with at least one textile yarn; removing the at least one textile yarn from the at least one elongated element to form a metallic reinforcing cord, wherein the at least one metallic wire extends in the metallic reinforcing cord along a helical path around a free space previously occupied by the at least one textile yarn; and

incorporating the metallic reinforcing cord in a piece of elastomeric material to make the structural component of the tyre, wherein the structural component is a carcass structure, a belt structure, a bead reinforcing structure, or a zero degrees belt layer of the tyre.

**2.** The process according to claim **1**, wherein providing the at least one elongated element comprises:

feeding the at least one metallic wire and the at least one textile yarn to a twisting device; and twisting together the at least one metallic wire and the at least one textile yarn in the twisting device to obtain the at least one elongated element.

## 36

**3.** The process according to claim **2**, further comprising, before removing the at least one textile yarn from the at least one elongated element:

winding the at least one elongated element on a respective service reel.

**4.** The process according to claim **2**, wherein removing the at least one textile yarn is carried out while the at least one elongated element is continuously fed.

**5.** The process according to claim **4**, wherein the at least one textile yarn is made of a water-soluble material, and wherein removing the at least one textile yarn comprises feeding a hot water jet against the at least one elongated element.

**6.** The process according to claim **5**, further comprising, after removing the at least one textile yarn:

drying the metallic reinforcing cord; and  
winding the metallic reinforcing cord on a collection reel.

**7.** The process according to claim **1**, wherein the at least one elongated element comprises at least two metallic wires twisted together with the at least one textile yarn.

**8.** The process according to claim **7**, wherein the metallic reinforcing cord comprises a plurality of cross sections, wherein the at least two metallic wires are in a condition of substantial mutual contact in said plurality of cross sections.

**9.** The process according to claim **8**, further comprising: deforming the metallic reinforcing cord so that in all of the cross sections thereof the at least two metallic wires are spaced apart from each other.

**10.** The process according to claim **9**, wherein deforming the metallic reinforcing cord comprises pulling the metallic reinforcing cord by a traction force, wherein the traction force is constant over time or variable over time.

**11.** The process according to claim **1**, wherein the at least one metallic wire has a diameter that ranges from 0.10 mm to 0.60 mm, the diameter being measured as prescribed by BISFA E10 method.

**12.** The process according to claim **1**, wherein the at least one metallic wire comprises a number of metallic wires that ranges from 1 to 27 metallic wires.

\* \* \* \* \*